



US007992989B2

(12) **United States Patent**  
**Makuta et al.**

(10) **Patent No.:** **US 7,992,989 B2**  
(b5) **Date of Patent:** **\*Aug. 9, 2011**

(54) **INK JET RECORDING METHOD AND INK JET RECORDING DEVICE**

(75) Inventors: **Toshiyuki Makuta**, Ashigarakami-gun (JP); **Yusuke Nakazawa**, Ashigarakami-gun (JP)

(73) Assignee: **Fujifilm Corporation**, Tokyo (JP)

(\*) Notice: Subject to any disclaimer, the term of this patent is extended or adjusted under 35 U.S.C. 154(b) by 946 days.

This patent is subject to a terminal disclaimer.

(21) Appl. No.: **11/896,268**

(22) Filed: **Aug. 30, 2007**

(65) **Prior Publication Data**

US 2008/0074482 A1 Mar. 27, 2008

(30) **Foreign Application Priority Data**

Sep. 25, 2006 (JP) ..... 2006-259356  
Mar. 30, 2007 (JP) ..... 2007-095505

(51) **Int. Cl.**

**B41J 2/175** (2006.01)

(52) **U.S. Cl.** ..... **347/100**; 347/96; 347/102; 106/31.13; 106/31.27; 106/31.6

(58) **Field of Classification Search** ..... 347/100, 347/102, 96; 106/31.13, 31.6, 31.27  
See application file for complete search history.

(56) **References Cited**

**U.S. PATENT DOCUMENTS**

6,007,182 A \* 12/1999 Matsubara et al. ..... 347/43  
7,645,036 B2 \* 1/2010 Umebayashi et al. ..... 347/100

|                   |        |                      |         |
|-------------------|--------|----------------------|---------|
| 2003/0021961 A1 * | 1/2003 | Ylitalo et al. ....  | 428/195 |
| 2004/0045931 A1   | 3/2004 | Hill et al.          |         |
| 2005/0065235 A1   | 3/2005 | Bauer                |         |
| 2005/0190248 A1   | 9/2005 | Konno et al.         |         |
| 2006/0023044 A1   | 2/2006 | Bauer                |         |
| 2006/0066704 A1 * | 3/2006 | Nishida .....        | 347/103 |
| 2006/0075917 A1 * | 4/2006 | Edwards .....        | 101/483 |
| 2006/0203056 A1 * | 9/2006 | Furukawa et al. .... | 347/96  |
| 2007/0216743 A1   | 9/2007 | Makuta et al.        |         |

**FOREIGN PATENT DOCUMENTS**

|                  |         |
|------------------|---------|
| EP 1 149 881 A2  | 10/2001 |
| EP 1 426 193 A1  | 6/2004  |
| EP 1 671 804 A1  | 6/2006  |
| EP 1 671 805 A2  | 6/2006  |
| JP 63-60783 A    | 3/1988  |
| JP 8-174997 A    | 7/1996  |
| JP 10-067905 A   | 3/1998  |
| JP 10-323975 A   | 12/1998 |
| JP 2003-145745 A | 5/2003  |
| JP 2004-42525 A  | 2/2004  |

(Continued)

*Primary Examiner* — Matthew Luu

*Assistant Examiner* — Rut Patel

(74) *Attorney, Agent, or Firm* — Sughrue Mion, PLLC

(57) **ABSTRACT**

An ink jet recording method comprising: applying an undercoating liquid containing an oligomer onto a recording medium; partially curing the undercoating liquid that has been applied onto the recording medium; and recording an image by ejecting an ink that is curable by irradiation of actinic energy onto the partially cured undercoating liquid. According to the invention, an image having excellent uniformity can be recorded on various types of recording media, irrespective of the type thereof, ink bleeding and unevenness in line width or color due to coalescence of ink droplets can be effectively suppressed, and an image with high density and a uniform dot diameter can be recorded when the image has low dot density such as low image resolution or image density.

**10 Claims, 9 Drawing Sheets**



FOREIGN PATENT DOCUMENTS

|    |             |    |         |
|----|-------------|----|---------|
| JP | 2004-42548  | A  | 2/2004  |
| JP | 2005-96254  | A  | 4/2005  |
| JP | 2005-154767 | A  | 6/2005  |
| JP | 2006-137183 | A  | 6/2006  |
| JP | 2006-137185 | A  | 6/2006  |
| WO | 02/085638   | A1 | 10/2002 |

|    |                |      |         |
|----|----------------|------|---------|
| WO | WO 2004/002746 | A1   | 1/2004  |
| WO | 2004/087824    | A2   | 10/2004 |
| WO | WO 2006046061  | A1 * | 5/2006  |
| WO | 2006/104278    | A1   | 10/2006 |
| WO | WO 2006128839  | A1 * | 12/2006 |

\* cited by examiner

Fig. 1A



Fig. 1B



Fig. 1C



Fig. 1D





Fig. 3A



Fig.3B



Fig. 4





Fig. 5

Fig. 6



Fig. 7A



Fig. 7B



Fig. 7C



Fig. 8



Fig. 9A



Fig. 9B



Fig. 9C



# INK JET RECORDING METHOD AND INK JET RECORDING DEVICE

## CROSS-REFERENCE TO RELATED APPLICATION

This application claims priority under 35 USC 119 from Japanese Patent Application Nos. 2006-259356 and 2007-95505, the disclosures of which are incorporated by reference herein.

## BACKGROUND OF THE INVENTION

### 1. Field of the Invention

The invention relates to an ink jet recording method and an ink jet recording device that are favorably used for formation of a high-quality image at high speed.

### 2. Description of the Related Art

An ink jet method of ejecting ink in the form of liquid droplets from an ink ejector has been used in various kinds of printers for the reasons of being compact and less expensive, capable of forming an image without contacting a recording medium, and the like. Among these ink jet methods, there are a piezo ink jet method utilizing deformation of piezoelectric elements to eject ink and a thermal ink jet method utilizing a boiling phenomenon of ink due to thermal energy to eject the ink in the form of droplets, which have the characteristics of high resolution and high-speed printability.

Improvements in speed and image quality have currently become important objectives, upon printing by ejecting ink droplets onto a plain paper sheet or a non-water absorbing recording medium made of plastics or the like with an ink jet printer.

Ink jet recording is a method of ejecting ink droplets according to image data to form a line or an image on a recording medium with the liquid droplets. However, there have been problems in practical use, particularly in a case of recording on the above-described non-absorbing recording medium, e.g., bleeding of an image easily occurs, or mixing of adjacent ink droplets occurs on the recording medium to inhibit formation of a sharp image, when it takes time for the liquid droplets to dry or penetrate into the recording medium after having been ejected. When the liquid droplets mix with each other, the ejected adjacent liquid droplets coalesce with each other to shift from the positions at which they have landed, thereby causing unevenness in line width in a case of forming fine lines or unevenness in color in a case of forming a colored area, or the like. Further, since the degree of occurrence of unevenness in line width or color unevenness in a colored area varies depending on ink absorption and wettability of the surface of the recording medium, there has also been a problem that different images are formed on different types of recording media, even when the same ink is used under the same ejection conditions.

As a method of suppressing image bleeding or nonuniformity of line width, there is a method of promoting fixation of liquid droplets. For example, there have been disclosed methods of using inks of two-liquid type having reactivity and allowing them to react with each other on a recording medium to achieve a depicting property with high definition, such as a method of recording with ink containing an anionic dye after application of a liquid containing a basic polymer (for example, refer to Japanese Patent Application Laid-Open (JP-A) No. 63-60783), or a method of applying ink containing an anionic compound and a coloring material after application of a liquid composition containing a cationic substance (for example, refer to JP-A No. 8-174997).

An ink jet recording method has also been proposed in which an ultraviolet-curable ink is used as the ink, the ink dots ejected onto a recording medium are irradiated with an ultraviolet ray in conformity with the timing of ejection, then the dots are pre-cured to be thickened to such an extent that the adjacent dots do not mix with each other, and thereafter the dots are further irradiated with ultraviolet rays to be completely cured (for example, refer to JP-A No. 2004-42548).

Further, a method has been proposed that improves visibility or remedies bleeding of color ink, or a problem such as variation in the obtained images formed on different types of recording media, by applying a radiation curable white ink to form a uniform undercoating layer on a transparent or semi-transparent non-absorbing recording medium, then curing or thickening the layer by irradiating with radiation rays, and thereafter recording with a radiation curable color ink (for example, refer to JP-A No. 2003-145745 and JP-A No. 2004-42525). There has also been proposed a method in which a substantially transparent active ray-curable ink is applied onto a recording medium in place of the above radiation curable white ink by an ink jet head (for example, refer to JP-A No. 2005-96254).

However, in the method described in JP-A No. 2004-42548, although bleeding can be suppressed, there still remains a problem of variation in images among various types of recording media, and thus a problem of unevenness in line width, color or the like due to mixing of ink droplets has not been sufficiently solved. This problem of unevenness in line width, color or the like due to mixing of ink droplets has also not been sufficiently solved by either of the methods described in JP-A No. 2003-145745 or JP-A No. 2004-42525. Further, there still remains a problem of unevenness in line width, color or the like due to mixing of ink droplets in the method described in JP-A No. 2005-96254.

On the other hand, when the ejected amount of an ink is small or the density of the ejected droplets is low, e.g., when an image is recorded by a head unit having low resolution in a single pass method by which an image can be formed at high speed, there are also problems in that disorders or bleeding in an image is caused by unregulated spreading of ink drops (dots), or to the contrary, white spots, degradation in density, bleeding or unevenness in an image is caused by insufficient spreading of the dots.

The invention has been made in view of the above problems and is intended to provide an ink jet recording method and an ink jet recording apparatus by which images having excellent uniformity can be recorded on various types of recording media and ink bleeding or unevenness in line width or color due to coalescence of ink droplets can be suppressed, and at the same time, an image can be well reproduced to details with high density while maintaining a uniform dot diameter, irrespective of the form of the image, when the image has low dot density such as low image resolution or image density and is recorded with a small amount of the ink.

The invention has been made based on the findings that it is important that the ejected and formed dots have the characteristics of spreading to a certain extent of area, and are capable of maintaining the shape thereof when the dots spread to coalesce with each other, in order to retain a high degree of density over the whole area of the image to details and allow reproduction of a clear image, in a case where the amount of the ink ejected at the time of recording is small and the dot density is relatively low.

When the dots spread to a desired extent, and the shapes thereof are maintained when they coalesce with each other, a certain degree of density can be achieved even when an image is recorded by a single pass method with a low-cost apparatus

provided with a head unit having low resolution, and also the quality of a recorded image can be improved.

#### SUMMARY OF THE INVENTION

The invention has been made in view of the above problems and provides an ink jet recording method and an ink jet recording device.

According to a first aspect of the invention, there is provided an ink jet recording method comprising:

applying an undercoating liquid containing an oligomer onto a recording medium;

partially curing the undercoating liquid that has been applied onto the recording medium; and

recording an image by ejecting an ink that is curable by irradiation of actinic energy onto the partially cured undercoating liquid.

According to a second aspect of the invention, there is provided an ink jet recording device comprising:

an undercoating liquid application unit that applies an undercoating liquid containing an oligomer onto a recording medium;

an undercoating liquid curing unit that is provided downstream of the undercoating liquid application unit and that partially cures the undercoating liquid by applying energy; and

an image recording unit that is provided downstream of the undercoating liquid curing unit and that forms an image by ejecting, onto the partially cured undercoating liquid, an ink that is curable by irradiation with actinic energy rays.

#### BRIEF DESCRIPTION OF THE DRAWINGS

Exemplary embodiments of the present invention will be described in detail based on the following figures, wherein:

FIGS. 1A to 1D are flow charts showing the mechanism of forming an image.

FIG. 2 is a schematic sectional view showing the entire configuration of an image recording device that records an image in accordance with the ink jet recording method of the invention;

FIG. 3A is a plan view showing an example of a basic entire structure of the ejecting head shown in FIG. 2;

FIG. 3B is a b-b line section of FIG. 3A;

FIG. 4 is a schematic view showing an exemplary configuration of a liquid supplying system that constitutes the image recording device;

FIG. 5 is a block diagram showing an exemplary configuration of a control system that constitutes the image recording device;

FIG. 6 is a schematic sectional view showing a state of ink droplets ejected onto a partially cured undercoating liquid;

FIGS. 7A and 7B are schematic sectional views showing a state that an ink is ejected onto an undercoating layer that has not been cured;

FIG. 7C is a schematic sectional view showing a state that an ink is ejected onto an undercoating liquid layer that has been completely cured;

FIG. 8 is a schematic sectional view showing a state of ink droplets B ejected onto a partially cured ink layer A;

FIGS. 9A and 9B are schematic sectional views showing a state that an ink B is ejected onto an ink layer A that has not been cured; and

FIG. 9C is a schematic sectional view showing a state that an ink B is ejected onto an ink layer A that has been completely cured.

#### DETAILED DESCRIPTION OF THE INVENTION

Details of the ink jet recording method and ink jet recording device of the invention will now be described.

The ink jet recording method of the invention includes the processes of applying an undercoating liquid containing an oligomer onto a recording medium; partially curing the applied undercoating liquid; and recording an image by ejecting, onto the partially cured undercoating liquid, an ink capable of being cured by irradiation with actinic energy rays. The method may further include other processes such as partially curing the ink, as necessary.

Generally, in an ink jet recording method, ink droplets are ejected so as to partly overlap each other in order to obtain a high degree of image density, and the adjacent ink droplets contact each other while staying on a recording medium, before being dried. Therefore, image bleeding or unevenness in line width of fine lines may easily occur due to the coalescence of the adjacent ink droplets to impair the formation of an image having high sharpness. However, according to the ink jet recording method of the invention, in which an undercoating liquid is applied onto a recording medium and partially cured, coalescence between the adjacent ink droplets can be suppressed by the interaction between the undercoating liquid and the ink droplets, even when the ink droplets are applied onto the partially cured undercoating liquid so as to partly overlap each other. Consequently, image bleeding, unevenness in line width of fine lines, or unevenness in a colored image can be effectively prevented.

Further, because of the oligomer contained in the undercoating liquid in the invention, ejected ink droplets spread to some degree to connect to each other but not so far as to impair the dot shape or cause image disorder or bleeding. Thus, an image can be formed that is clearly reproduced to details, while retaining a high degree of density over the whole image and preventing white spots, when the image is recorded with a head unit with low resolution in a single pass method or a part of the image with low dot density (such as an image with low density or low resolution) is recorded with a small liquid amount.

Therefore, according to the ink jet recording method of the invention, sharp lines with a uniform width can be formed and reproducibility of a fine image such as a fine line in an image can be improved without causing white spots or reduction in density, even when the recording is performed with a small liquid amount and low dot density.

The ink jet recording method of the invention is effective in the cases where an image is recorded on a non-permeable or slowly permeable recording medium having low liquid absorbability, and especially effective in the cases where an image is recorded with a low-cost head unit having low resolution, such as 300 dpi or less, in a single pass image recording method.

In the invention, the description "adjacent ink droplets" refers to liquid droplets of an ink of a single color ejected from an ink ejecting port so as to have an overlapping portion, or liquid droplets of inks of different colors respectively ejected from respective ink ejecting ports so as to have an overlapping portion. The adjacent ink droplets may be the liquid droplets that are ejected at the same time, or may be a combination of preceding liquid droplets and following liquid droplets where the former are ejected prior to the ejection of the latter.

In the invention, at least one kind of ink and at least one kind of undercoating liquid are used as the liquids for formation of an image. The undercoating liquid preferably has a different composition from that of the ink. The undercoating liquid is preferably applied onto the region that is equal to, or

larger than, the region on which an image is to be formed by ejecting ink droplets onto a recording medium.

Further, the ink in the invention is preferably used as inks of plural colors in a multicolor ink set. In a case of using the multicolor ink set, it is preferable that after each ejection of the ink of each color, partially curing the ink droplets is further performed.

One of the specific configurations of the ink jet recording method of the invention includes the steps of applying, onto a recording medium, an undercoating liquid containing a polymerizable or crosslinkable material, in advance in the region that is equal to, or larger than, the region on which an image is formed with ink; applying energy rays or heat to the undercoating liquid applied onto the recording medium to half-cure the undercoating liquid; and after partially curing the undercoating liquid, ejecting ink droplets of plural colors onto the undercoating liquid that has been applied onto the recording medium, wherein the ink droplets contain a polymerizable or crosslinkable material for formation of the image and have a different composition from that of the undercoating liquid.

In the above method, it is preferable to provide a step of fixing the recorded image to further promote the curing of the undercoating liquid and the ink by applying energy and the like (hereinafter, referred to as fixing process), after the undercoating liquid has been applied and at least all of the desired ink (preferably inks of plural colors) have been ejected, from the viewpoint of achieving excellent fixing properties against the ink.

#### -Application of Undercoating Liquid and Recording-

In the undercoating liquid application process, an undercoating liquid is applied onto a recording medium. The undercoating liquid contains at least an oligomer, and preferably contains a radical polymerizable compound and a surfactant. The undercoating liquid may further include other components. Details of the components that constitute the undercoating will be discussed later.

In the recording process, an image is recorded by ejecting an ink that is curable by irradiation with actinic energy rays onto a partially cured undercoating liquid that has been partially cured in a partial curing process to be described later. The ink is applied onto the partially cured undercoating liquid in the form of droplets by using an ink jet nozzle or the like.

In the ink jet recording method of the invention, the undercoating liquid can be applied onto the recording medium using a coating device, an ink jet nozzle, and the like.

#### (i) Application Using an Application Device

In a preferable embodiment of the invention, image recording is performed by applying an undercoating liquid onto a recording medium using an application device, and thereafter ink droplets are ejected using an ink jet nozzle. Details of the ink jet nozzle will be discussed later.

The application device is not particularly limited and can be selected from known application devices as appropriate according to purposes. Examples of the application devices include an air doctor coater, blade coater, lot coater, knife coater, squeeze coater, immersion coater, reverse roll coater, transfer roll coater, gravure coater, kiss roll coater, cast coater, spray coater, curtain coater and an extruding coater. Details of these coating devices are described in Yuji Harasaki, "Coating Engineering", (1978).

#### (ii) Ejection by Ink Jet Nozzle

In the invention, an embodiment is also preferable in which an image is recorded by ejecting an undercoating liquid using an ink jet nozzle, and thereafter ink droplets are ejected by an ink jet nozzle. Details of the ink jet nozzle will be discussed later.

As the conditions for applying of the undercoating liquid by the ink jet nozzle, it is preferable that the undercoating liquid is ejected by a head capable of ejecting a greater amount per droplet and having lower nozzle density as compared with the head for an ink, and the head is arranged as a full-line head unit in a width direction of the recording medium. Such a head having a greater amount per droplets to be ejected generally has a high degree of ejection power, and is therefore compatible with an undercoating liquid having high viscosity, and is also advantageous in terms of avoiding nozzle clogging. Further, using of a head capable of ejecting a greater amount per droplet is also advantageous from the viewpoint that a low-cost head having low driving frequency can be applied, since the droplet resolution of the undercoating liquid in a direction in which a recording medium is conveyed can be reduced.

In either case of the above embodiments, liquids other than the undercoating liquid and ink can be further applied. Any means such as an application device or an ink jet nozzle can be used for the application of such liquids, and the timing thereof is also not particularly limited. When a colorant is contained in the liquid other than the undercoating liquid and ink, the liquid is preferably applied by ejecting with an ink jet nozzle, and is preferably applied after the undercoating liquid has been applied.

Next, a method of ejecting using an ink jet nozzle (ink jet recording method) will be discussed.

In the invention, known ink jet recording methods are preferably used, such as an electrostatic induction method in which an ink is ejected by means of electrostatic power, drop-on-demand method (pressure-pulse method) utilizing vibration pressure of a piezoelectric element, acoustic ink jet method in which ink is ejected by means of radiation pressure caused by irradiating the ink with an acoustic beam which has been converted from an electric signal, and a thermal ink jet method of utilizing pressure generated by heating ink to form air bubbles.

In the invention, the ink is preferably ejected onto the partially cured undercoating liquid to a droplet size of from 0.1 pL (picoliter; hereinafter the same) to 100 pL. When the droplet size is within the above range, an image with high sharpness and density can be effectively formed. The droplet size is more preferably in the range of from 0.5 pL to 50 pL.

The amount of the undercoating liquid to be applied in terms of mass ratio per area is preferably from 0.05 to 5, more preferably from 0.07 to 4, and still more preferably from 0.1 to 3.

The ejection interval between the application of the undercoating liquid and the ejection of the ink droplets is preferably in the range of from 5μ seconds to 10 seconds. When the ejection interval is within the above range, the effect of the invention can be remarkably achieved. The ejection interval of the ink droplet is more preferably in the range of from 10μ seconds to 5 seconds, and particularly preferably from 20μ seconds to 5 seconds.

Further, in the recording process, a multicolored image can be recorded using an ink set including inks of multiple colors. In this case, in terms of reproducibility of a fine image or color tone, it is preferable to provide a step of partially curing at least one of the inks of multiple colors ejected onto a recording medium, and an exposure process (so-called pinning exposure) after each ejection of the ink of one color or a predetermined set of colors.

Actinic energy rays are preferably used for the pinning exposure and details thereof is the same as the cases in the fixing process to be described later. Examples of the actinic energy rays include ultraviolet rays, visible rays, α-rays,

$\gamma$ -rays, X-rays and electron rays. Among these, ultraviolet rays and visible rays are preferable in terms of cost and safety, and ultraviolet rays are most preferable.

The amount of the energy required for partially curing here varies depending on the type or content of a polymerization initiator, but is generally preferably from 1 to 500 mJ/cm<sup>2</sup>, more preferably from 1 to 200 mJ/cm<sup>2</sup>, and still more preferably from 1 to 100 mJ/cm<sup>2</sup>.

-Curing Process-

In the curing process, the undercoating liquid that has been applied in the above-described application process is partially cured.

In the invention, the curing process is provided after the application of the undercoating liquid and before the ejection of at least one ink.

In the invention, the expression "partially curing" refers to a state in which the undercoating liquid is partially but not completely cured. When the undercoating liquid that has been applied onto a recording medium (substrate) is partially cured, the degree of the curing may be uneven. For example, the curing is preferably more developed at a deeper point in a depth direction.

When a radical polymerizable undercoating liquid is used in the air or the air that has partly substituted by an inert gas, the radial polymerization at the surface of the undercoating liquid tends to be inhibited by the action of oxygen to inhibit the radial polymerization. As a result, the degree of the curing becomes uneven and the curing tends to be more developed in the inside of the undercoating liquid than at the surface thereof. In a case where a cationic polymerization liquid is used in the air containing moisture, the curing also tends to be more developed in the inside of the undercoating liquid than at the surface thereof, due to the action of the moisture to inhibit the cationic polymerization.

In the invention, when a radical photopolymerizable undercoating liquid is used under coexistence of oxygen that tends to inhibit radical polymerization and partially photo-cured, the curing degree of the undercoating liquid becomes higher at the outside than in the inside thereof.

When an ink (hereinafter, referred to as "colored liquid" sometimes) is ejected onto an undercoating liquid that has not been cured, favorable effects can be achieved in the quality of an image that has been formed onto a recording medium. The mechanism of this action can be determined by observing a section of the recording medium.

Hereinafter, explanation will be given taking the case where an ink of about 12 pL is ejected onto a partially cured undercoating liquid layer having a thickness of 5  $\mu$ m as an example.

In the invention, an undercoating liquid is partially cured and the degree of curing thereof is higher at a point that is closer to a substrate, relative to that at a point farther from the substrate. In this case, three features can be observed: that is, as shown in FIG. 6, (1) a part of an ink 24 is exposed on the surface; (2) a part of the ink 24 is submerged in an undercoating layer 20; and (3) the undercoating liquid 20 exists between the ink 24 and the substrate 26. Therefore, the recording medium on which an image is formed by applying the ink 24 onto the partially cured undercoating layer 20 has a section as schematically shown in FIG. 6. In a case where all of the above conditions (1), (2) and (3) are satisfied, it can be determined that the ink 24 has been applied onto the undercoating layer 20 which is in a partially cured state. In this case, the colored droplets that have been ejected with high density coalesce with each other to form a colored film, and a uniform and high degree of color density can be achieved.

On the other hand, as shown in FIGS. 7A and 7B, when the ink 24 is ejected onto the undercoating liquid 20 that has not been cured, the ink 24 submerges entirely in the undercoating liquid 20, and/or the undercoating liquid 20 does not exist between the ink 24 and the substrate 26. In this case, the droplets remain independent from each other even when the ink is applied with high density, thereby becoming a factor of reduced color density. The recording medium on which an image is formed by applying the ink 24 onto the uncured undercoating liquid 20 has a section as schematically shown in FIGS. 7A and 7B.

When the ink 24 is ejected onto a completely cured undercoating liquid 20, the ink 24 does not submerge in the undercoating liquid 20, as shown in FIG. 7C. Such a situation may become a factor of interdroplet interference, thereby failing to form a uniform ink film and causing reduction in color reproducibility. The recording medium on which an image is formed by applying the ink 24 onto the completely cured undercoating liquid 20 has a section as schematically shown in FIG. 7C.

It is preferable that the amount per area of the uncured part of the undercoating liquid is sufficiently smaller than the largest amount per area of the applied ink, from the viewpoint that when the ink droplets are applied with high density, they do not remain independent of each other and form a uniform liquid layer of the ink; and that the occurrence of interdroplet interference is prevented. Therefore, the mass per area of the uncured part of the undercoating liquid "M (undercoating liquid)" and the largest mass per area of the applied ink droplets "m (ink)" preferably satisfies a relation "m (ink)/30 < M (undercoating liquid) < m (ink)", further preferably satisfies a relation "m (ink)/20 < M (undercoating liquid) < m (ink)/3", and still more preferably satisfies a relation "m (ink)/10 < M (undercoating liquid) < m (ink)/5". The largest mass per area of the ink to be ejected here refers to the largest mass of each case of respective colors. When a relation "m (ink)/30 < M (undercoating liquid)" is satisfied, occurrence of interdroplet interference can be prevented and excellent dot size reproducibility can be achieved. Further, when a relation "M (undercoating liquid) < m (ink)" is satisfied, uniform liquid layer of the ink can be formed and high density can be obtained.

The mass per area of the uncured part of the undercoating liquid can be determined by a transferring test, in which a permeable medium such as a plain paper sheet is pressed against the partially cured undercoating liquid, at a point after the completion of the partially curing process (e.g., after irradiation with actinic energy rays) and prior to the ejection of the ink droplets, and the mass of the undercoating liquid that has been transferred onto the permeable medium from the undercoating layer is measured.

For example, when the largest ejection amount of the ink droplets in an ejection density of 600×600 dpi is 12 pL per pixel, the largest mass per area of the ejected ink "m (ink)" is determined to be 7.4 g/cm<sup>2</sup> (here, the density of the ink is assumed to be 1.1 g/cm<sup>3</sup>). Therefore, the preferable mass per area of the uncured part of the undercoating liquid is greater than 0.25 g/cm<sup>2</sup> and less than 7.4 g/cm<sup>2</sup>, more preferably greater than 0.37 g/cm<sup>2</sup> and less than 2.5 g/cm<sup>2</sup>, and still more preferably greater than 0.74 g/cm<sup>2</sup> and less than 1.48 g/cm<sup>2</sup>.

Further, in a case of forming a secondary color from the inks of two colors (hereinafter, referred to as an ink A and an ink B), one of the inks can be applied onto the other ink that has been partially cured, e.g., applying the ink B onto the partially cured ink A. When the ink B is ejected onto the partially cured ink A, a part of the ink B28 submerges in the ink A24, and at the same time, the ink A24 exists under the ink

B28. Therefore, a recording medium on which an image is formed by applying the ink B28 onto the partially cured ink A24 has a section as schematically shown in FIG. 8. By laminating the cured layers of the inks A and B, favorable color reproduction can be achieved.

On the other hand, when the ink B is ejected onto the uncured ink A, the ink B28 submerges entirely in the ink A24, as shown in FIG. 9A, and/or the ink A24 does not exist under the ink B28, as shown in FIG. 9B. In this case, the droplets remain independent from each other even when the ink B is applied with high density, thereby becoming a factor of reduced color saturation of the secondary color. The recording medium on which an image is formed by applying the ink B28 onto the uncured ink A24 thus has a section as schematically shown in FIGS. 9A and 9B.

When the ink B is ejected onto the completely cured ink A, ink B28 does not submerge in the ink A24, as shown in FIG. 9C. Such a situation may become a factor of interdroplet interference, thereby failing to form a uniform ink film and causing reduction in color reproducibility. The recording medium on which an image is formed by applying the ink B28 onto the completely cured ink A24 thus has a section as schematically shown in FIG. 9C.

It is preferable that the amount per area of the uncured part of the ink A is sufficiently smaller than the largest amount per area of the applied ink B, from the viewpoint that the droplets of the ink B applied with high density does not remain independent of each other and form a uniform liquid layer of ink B, and that occurrence of interdroplet interference is prevented. Therefore, the mass per area of the uncured part of ink A layer "M (ink A)" and the largest mass per area of the applied droplets of the ink B "m (ink B)" preferably satisfies a relation " $m (ink B)/30 < M (ink A) < m (ink B)$ ", further preferably satisfies a relation " $m (ink B)/20 < M (ink A) < m (ink B)/3$ ", and still more preferably satisfies a relation " $m (ink B)/10 < M (ink A) < m (ink B)/5$ ". When a relation " $m (ink B)/30 < M (ink A)$ " is satisfied, occurrence of interdroplet interference can be prevented, and excellent dot size reproducibility can be achieved. Further, when a relation " $M (ink A) < m (ink B)$ " is satisfied, uniform liquid layer of an ink can be formed and high density can be obtained.

The mass per area of the uncured part of the ink A can be determined by a transferring test, in which a permeable medium such as a plain paper sheet is pressed against the partially cured layer of ink A, at a point after the completion of the partial curing process (e.g., after irradiation with actinic energy rays) and prior to the ejection of the droplets of ink B, and the mass of the liquid that has been transferred onto the permeable medium from the layer of the ink A is measured.

For example, when the largest ejection amount of the droplets of the ink B in an ejection density of 600×600 dpi is 12 pL per pixel, the largest mass per area of the ejected ink B "m (ink)" is determined to be 7.4 g/cm<sup>2</sup> (here, the density of the ink B is assumed to be 1.1 g/cm<sup>3</sup>). Therefore, the mass per area of the uncured part of the layer of the ink A is preferably greater than 0.25 g/cm<sup>2</sup> and less than 7.4 g/cm<sup>2</sup>, more preferably greater than 0.37 g/cm<sup>2</sup> and less than 2.5 g/cm<sup>2</sup>, and still more preferably greater than 0.74 g/cm<sup>2</sup> and less than 1.48 g/cm<sup>2</sup>.

When the curing reaction is based on an ethylene unsaturated compound or a cyclic ether, the unpolymerization rate can be quantitatively measured from the reaction rate of an ethylene unsaturated group or a cyclic ether group (discussed later).

When the above-described partially cured state of the undercoating liquid and/or the ink is achieved by polymerization reaction of a polymerizable compound that starts

polymerization by irradiation with actinic energy rays or heating, the unpolymerization rate defined as "A (after polymerization)/A (before polymerization)" is preferably from 0.2 to 0.9, more preferably from 0.3 to 0.9, and still more preferably from 0.5 to 0.9, in terms of improving abrasion resistance of a printed material.

In the above discussion, "A (after polymerization)" indicates an absorbance at an infrared absorption peak of a polymerizable group after polymerization, and "A (before polymerization)" indicates an absorbance at an infrared absorption peak of a polymerizable group before polymerization. For example, when the polymerizable compound contained in the undercoating liquid and/or the colored liquid is an acrylate monomer or a methacrylate monomer, an absorption peak based on a polymerizable group (acrylate group or methacrylate group) can be observed in the vicinity of 810 cm<sup>-1</sup>, and the unpolymerization rate is preferably determined by the absorbance at this peak. On the other hand, when the polymerizable compound is an oxetane compound, an absorption peak based on a polymerizable group (oxetane group) can be observed in the vicinity of 986 cm<sup>-1</sup>, and the unpolymerization rate is preferably determined by the absorbance at this peak. Further, when the polymerizable compound is an epoxy compound, an absorption peak based on a polymerizable group (epoxy group) can be observed in the vicinity of 750 cm<sup>-1</sup>, and the unpolymerization rate is preferably determined by the absorbance at this peak.

As the device for measuring of an infrared absorption spectrum, any commercially available infrared spectrometer of transmission type or reflection type may be used and selected according to the form of the sample. For example, an infrared spectrometer (FTS-6000, manufactured by BIO-RAD Laboratories, Inc.) can be used for the measurement.

Further preferable partially cured state can be determined by observing the section of ink droplet that has been ejected onto a partially cured undercoating liquid. The method of observation is not particularly limited, but for example, a commercially available microtome or optical microscope can be used. The size of the ink droplet ejected onto a partially cured undercoating liquid is preferably in the range of from 1 pL to 100 pL, and is further preferably equal to the size of the ink droplet which is practically used. Further, the partially cured film is preferably hardened by a method of some kind, at the time of observation. The method for hardening is not particularly limited, but may be a method of utilizing freezing, polymerization or the like.

The methods for partially curing the undercoating layer can be exemplified by known methods for increasing viscosity, such as: (1) a method of utilizing a so-called aggregation phenomenon performed by adding a basic compound to an acidic polymer, or adding an acidic compound or metallic compound to a basic polymer; (2) a method of adjusting the viscosity of the undercoating liquid or white ink by preliminarily preparing an undercoating liquid to have high viscosity, then adding a low boiling point organic solvent to the undercoating liquid to decrease the viscosity thereof, and thereafter bringing the undercoating liquid back to have high viscosity by evaporating the low boiling point organic solvent; (3) a method of adjusting the viscosity of the undercoating liquid or white ink by heating the undercoating liquid which has previously been prepared to have high viscosity, then cooling the undercoating liquid back to have high viscosity; and (4) a method of causing a curing reaction by applying actinic energy rays or heat to the undercoating liquid or white ink. Among these, (4) a method of causing a curing reaction by applying actinic energy rays or heat to the undercoating liquid or white ink is most preferable.

## 11

The method of causing a curing reaction by applying actinic energy rays or heat to an undercoating liquid or white ink is a method of causing an insufficient polymerization reaction of a polymerizable compound at the surface of the undercoating liquid applied onto a recording medium. At the surface of the undercoating layer, the polymerization reaction is easily inhibited under the influences of oxygen in the air, as compared with the inside of the undercoating layer. Therefore, partially curing the undercoating layer can be caused by regulating the conditions of application of actinic energy rays or heat.

The amount of the energy required for partially curing the undercoating liquid varies depending on the type or content of the polymerization initiator, but is generally preferably from about 1 to about 500 mJ/cm<sup>2</sup> when energy is applied by actinic energy rays. When energy is applied by heating, it is preferable to heat a recording medium under the conditions where the surface temperature of the recording medium becomes in the range of from 40 to 80°C., for a period of from 0.1 to 1 second.

By applying actinic energy rays or heat such as active light or heat, generation of active species can be promoted by decomposition of the polymerization initiator, and the curing reaction due to polymerization or crosslinking of a polymerizable or crosslinkable material resulting from the active species can be promoted, by the increased active species or elevated temperature. Increasing of viscosity can also be favorably performed by irradiating with active light or heating.

In the above, partially curing the undercoating liquid has been discussed, but the same will apply to the cases of partially curing the ink.

The viscosity of the internal partially cured undercoating liquid (25°C.) is preferably 5000 mPa·s or more. The viscosity at the surface of the partially cured undercoating liquid (25°C.) is preferably 100 mPa·s or more and less than 5000 mPa·s. The viscosities at the surface and at the internal portion can be measured by a commercially available viscometer (e.g., a portable digital viscometer for laboratory use, VISCOSTICK, manufactured by MARUYASU INDUSTRIES Co., Ltd.), using samples obtained by scraping up the surface and internal portion of the partially cured undercoating liquid (25°C.), respectively.

Further, the viscosity of the internal portion of the partially cured undercoating liquid (25°C.) is preferably at least 1.5 times as high as, more preferably at least 2 times as high as, and still more preferably at least 3 times as high as that of the surface portion of the partially cured undercoating liquid (25°C.) from the viewpoint of suppressing coalescence between adjacent ink droplets due to interaction of the undercoating liquid and the ink droplets.

The degree of polymerization of the polymerizable compound at the surface of the partially cured undercoating liquid is preferably from 1% to 70%, more preferably from 5% to 60%, and still more preferably from 10% to 50%. The degree of polymerization can be measured by IR or the like.

Details of the actinic energy rays are the same as those to be described later and examples thereof include ultraviolet rays, visible rays,  $\alpha$  rays,  $\gamma$  rays, X rays and electron beams, wherein ultraviolet rays and visible rays are preferable, and ultraviolet rays are particularly preferable, from the viewpoint of cost and safety.

## -Fixing Process-

A fixing process is preferably carried out after the processes of above discussed undercoating liquid application, curing and recording. In the fixing process, curing of the

## 12

undercoating liquid and ejected ink is further promoted by applying energy or the like, thereby fixing the recorded image.

When a polymerizable or crosslinkable material is contained in the image, the curing reaction can be promoted due to the polymerization or crosslinking of the material by applying energy, and therefore a stronger image can be formed with higher efficiency. For example, in a system containing a polymerization initiator, generation of active species due to the decomposition of the polymerization initiator is promoted by the application of actinic energy, such as actinic energy rays, or heating, and the curing reaction is promoted by the polymerization or crosslinking of polymerizable or crosslinkable material due to the active species, by the increased amount of active species or elevated temperature.

Application of energy can favorably be performed by irradiating with actinic energy rays or heating. As the actinic energy, similar ones to the later discussed active lights for image fixation can be used, such as ultraviolet rays, visible rays,  $\alpha$ -rays,  $\gamma$ -rays, X-rays and electron beams, wherein ultraviolet rays and visible rays are preferable and ultraviolet rays are particularly preferable, from the viewpoint of cost or safety.

The heating can be performed using a non-contact type heating device, and preferable examples thereof include a heating device that allows a recording medium to pass through the inside of a heating chamber such as an oven, or a heating device that performs a whole-area exposure over a recording medium with light of ultraviolet light-visible light-infrared light, or the like. Examples of the preferable light sources for use in exposure as a heating device include a metal halide lamp, xenon lamp, tungsten lamp, carbon arc lamp and a mercury lamp.

When the energy is applied by irradiation with active light, the amount of the energy required for curing reaction varies depending on the type or content of the polymerization initiator, but is generally preferably from about 100 to about 10,000 mJ/cm<sup>2</sup>. When the energy is applied by heating, it is preferable to heat a recording medium under such conditions that the surface temperature of the recording medium becomes from 40 to 80°C., for the period of from 0.1 to 1 second.

## (Curing Sensitivity of Ink and Undercoating Liquid)

In the invention, the curing sensitivity of the ink is preferably equal to or higher than the curing sensitivity of the undercoating liquid. More preferably, the curing sensitivity of the ink is not less than the curing sensitivity of the undercoating liquid and not more than ten times as high as the curing sensitivity of the undercoating liquid, and still more preferably the curing sensitivity of the ink is not less than the curing sensitivity of the undercoating liquid and not more than five times as high as the curing sensitivity of the undercoating liquid. Further preferably, the curing sensitivity of the ink is not less than the curing sensitivity of the undercoating liquid and not more than twice as high as the curing sensitivity of the undercoating liquid or less.

The curing sensitivity here refers to the amount of the energy necessary to completely cure the ink and/or the undercoating liquid using a mercury lamp of super high pressure, high pressure, medium pressure or the like, preferably a super high pressure mercury lamp. Smaller amount of the necessary energy indicates that the sensitivity is higher. Therefore, the curing sensitivity being twice as high indicates that the amount of energy is  $1/2$  as much.

When one of the two curing sensitivities is not more than twice as high as the other, the two curing sensitivities are regarded as being equal.

## 13

(Physical Properties of Ink and Undercoating Liquid)

Regarding the physical properties of the ink (liquid droplets) to be ejected onto a recording medium by an ink jet recording method, the viscosity thereof at 25°C. is preferably in the range of from 5 to 100 mPa·s, and more preferably in the range of from 10 to 80 mPa·s, although the value may vary dependent on the type of the devices. The viscosity at 25°C. of the undercoating liquid before being subjected to partial curing is preferably in the range of from 100 to 5,000 mPa·s, and more preferably in the range of from 200 to 3,000 mPa·s.

In the invention, the undercoating liquid preferably contains a surfactant from the viewpoint of forming dots of desired size onto a recording medium, and preferably satisfies all of the conditions (A), (B), and (C) described below:

(A) The surface tension of the undercoating liquid is smaller than that of at least one of the inks.

(B) At least one surfactant contained in the undercoating liquid satisfies the following relation:

$$\gamma_s(0) - \gamma_s(\text{saturated}) > 0 \text{ (mN/m)}$$

(C) The surface tension of the undercoating liquid satisfies the following relation:

$$\gamma_s < (\gamma_s(0) + \gamma_s(\text{saturated})^{max})/2$$

In the above relations,  $\gamma_s$  is the value of the surface tension of the undercoating liquid;  $\gamma_s(0)$  is the value of the surface tension of the liquid having a composition of the undercoating liquid from which all surfactants are excluded;  $\gamma_s(\text{saturated})$  is the value of the surface tension of the liquid, wherein the liquid is obtained by adding one of the surfactants contained in the undercoating liquid to the above "liquid excluding all of the surfactants", the value being measured when the surface tension reaches a point of saturation as the density of the surfactant is increased; and  $\gamma_s(\text{saturated})^{max}$  is the maximum value among the values of  $\gamma_s(\text{saturated})$  respectively measured for all kinds of the surfactants which are contained in the undercoating liquid that satisfy the above condition (B).

<Condition (A)>

In the invention, the surface tension  $\gamma_s$  of the undercoating liquid is preferably smaller than the surface tension  $\gamma_k$  of at least one of the inks in order to form ink dots of desired size onto the recording medium as described above.

Further, from the viewpoint of preventing the spreading of the ink dots during the period from the landing of the ink droplets up to the exposure more effectively, the values of  $\gamma_s$  and  $\gamma_k$  preferably satisfy the relation of  $\gamma_s < \gamma_k - 3 \text{ (mN/m)}$ , and more preferably satisfy the relation of  $\gamma_s < \gamma_k - 5 \text{ (mN/m)}$ .

In a case of printing a full-color image, from the viewpoint of improving sharpness of the image, the surface tension of the undercoating liquid  $\gamma_s$  is preferably at least smaller than the surface tension of the ink containing a coloring agent with high visibility, and more preferably smaller than the surface tensions of all of the inks. The coloring agent with high visibility is, for example, a coloring agent that exhibits the color of magenta, black, or cyan.

Even though the values of the surface tension of the ink  $\gamma_k$  and the surface tension of the undercoating liquid  $\gamma_s$  satisfy the above-described relations, when both of the values are less than 15 mN/m, formation of the liquid droplets may become difficult at the time of ejecting the ink, and the ejection may not be carried out. On the other hand, when the above values are greater than 50 mN/m, wettability with the

## 14

ink jet head may be deteriorated to cause a failure in ejection. Therefore, it is preferable that each of the surface tension of the ink  $\gamma_k$  and the surface tension of the undercoating liquid  $\gamma_s$  is within the range of from 15 mN/m to 50 mN/m, more preferably in the range of from 18 mN/m to 40 mN/m, and particularly preferably in the range of from 20 mN/m to 38 mN/m.

The surface tension mentioned here is a value measured in accordance with a Wilhelmy method at a liquid temperature of 20°C. and at 60% RH, by a commonly used surface tensiometer (for example, surface tensiometer CBVP-Z, manufactured by Kyowa Interface Science Co., Ltd.).

<Conditions (B) and (C)>

In the invention, the undercoating liquid preferably contains at least one kind of surfactant in order to form the ink dots of desired size onto a recording medium. In this case, it is preferable that at least one kind of surfactant contained in the undercoating liquid satisfies the condition (B) described below:

$$\gamma_s(0) - \gamma_s(\text{saturated}) > 0 \text{ (mN/m)} \quad \text{Condition (B)}$$

Further, it is preferable that the surface tension of the undercoating liquid preferably satisfies the condition (C) described below:

$$\gamma_s < (\gamma_s(0) + \gamma_s(\text{saturated})^{max})/2 \quad \text{Condition (C)}$$

As mentioned above,  $\gamma_s$  is the value of the surface tension of the undercoating liquid;  $\gamma_s(0)$  is the value of the surface tension of the liquid having a composition of the undercoating liquid from which all surfactants are excluded;  $\gamma_s(\text{saturated})$  is the value of the surface tension of the liquid, wherein the liquid is obtained by adding one kind of the surfactants contained in the undercoating liquid to the above "liquid excluding all of the surfactants", and wherein the value is measured when the surface tension reaches a point of saturation as the density of the surfactant is increased; and  $\gamma_s(\text{saturated})^{max}$  is the maximum value among the values of  $\gamma_s(\text{saturated})$  respectively measured for all kinds of surfactants contained in the undercoating liquid that satisfy the above condition (B).

The value  $\gamma_s(0)$  can be obtained by measuring the value of the surface tension of the liquid having the composition of the undercoating liquid from which all surfactants are excluded. The value  $\gamma_s(\text{saturated})$  can be obtained by adding one kind of the surfactant contained in the undercoating liquid to the "liquid excluding all of the surfactants", then increasing the concentration of the surfactant by the increment of 0.01% by mass, and measuring the surface tension at the point where the change in the degree of the surface tension relative to the change in the concentration of the surfactant becomes 0.01 mN/m or less.

Details of the values  $\gamma_s(0)$ ,  $\gamma_s(\text{saturated})$  and  $\gamma_s(\text{saturated})^{max}$  will be discussed below by reference with the case where components of the undercoating liquid (Example 1) are: a high boiling point solvent (diethyl phthalate, manufactured by Wako Pure Chemical Industries, Ltd.); a polymerizable material (dipropylene glycol diacrylate, manufactured by Akros Chemicals Ltd.), a polymerization initiator (TPO, shown below as "Initiator-1"); a fluorine-based surfactant (MEGAFAC F475, manufactured by Dainippon Ink and Chemicals, Inc.); and a hydrocarbon-based surfactant (sodium di-2-ethylhexyl sulfosuccinate).



Initiator-1

In the above example, the values of  $\gamma_s(0)$ ,  $\gamma_s$  (saturated)<sup>1</sup> (when the fluorine-based surfactant is added),  $\gamma_s$  (saturated)<sup>2</sup> (when the hydrocarbon-based surfactant is added),  $\gamma_s$  (saturated), and  $\gamma_s$  (saturated)<sup>max</sup> are determined as follows.

The value of  $\gamma_s(0)$ , indicating the surface tension of the liquid having a composition of the undercoating liquid from which all surfactants are excluded, is determined as 36.7 mN/m.

The value of  $\gamma_s$  (saturated)<sup>1</sup>, which is the saturated value of the surface tension of the liquid when the fluorine-based surfactant is added and the concentration thereof is increased, is determined as 20.2 mN/m.

The value of  $\gamma_s$  (saturated)<sup>2</sup>, which is the saturated value of the surface tension of the liquid when the hydrocarbon-based surfactant is added and the concentration thereof is increased, is determined as 30.5 mN/m.

Since the undercoating liquid (Example 1) contains two kinds of the surfactants that satisfy the above-described condition (B), there are two values of  $\gamma_s$  (saturated), i.e., the value when the fluorine-based surfactant is added ( $\gamma_s$  (saturated)<sup>1</sup>) and the value when the hydrocarbon-based surfactant is added ( $\gamma_s$  (saturated)<sup>2</sup>). Here, the value of  $\gamma_s$  (saturated)<sup>max</sup>, i.e., the maximum value between  $\gamma_s$  (saturated)<sup>1</sup> and  $\gamma_s$  (saturated)<sup>2</sup>, is determined as the value of  $\gamma_s$  (saturated)<sup>2</sup>.

The above results are summarized as follows:

$$\gamma_s(0) = 36.7 \text{ mN/m}$$

$\gamma_s$  (saturated)<sup>2</sup> = 20.2 mN/m (when the fluorine-based surfactant is added)

$\gamma_s$  (saturated)<sup>2</sup> = 30.5 mN/m (when the hydrocarbon-based surfactant is added)

$$\gamma_s$$
 (saturated)<sup>max</sup> = 30.5 mN/m

From the above results, the surface tension of the undercoating liquid  $\gamma_s$  preferably satisfies the relationship:

$$\gamma_s < (\gamma_s(0) + \gamma_s(\text{saturated})^{max})/2 = 33.6 \text{ mN/m.}$$

As for the above-described condition (C), from the viewpoint of preventing spreading of the ink droplets during the period from the landing of the liquid droplets up to the exposure, the surface tension of the undercoating liquid more preferably satisfies the relationship:

$$\gamma_s < \gamma_s(0) - 3 \times \{\gamma_s(0) + \gamma_s(\text{saturated})^{max}\}/4$$

and particularly preferably satisfies the relationship:

$$\gamma_s \leq \gamma_s(\text{saturated})^{max}$$

The compositions of the ink and the undercoating liquid may be selected so that the desired surface tension can be obtained, but it is preferable that these liquids contain a surfactant. As described above, in order to form the ink dots of desired size onto a recording medium, the undercoating liquid preferably contains at least one kind of surfactant. The following are the details of the surfactants.

#### (Surfactant)

The surfactant in the invention is a substance having strong surface activity to at least one solvent selected from hexane, cyclohexane, p-xylene, toluene, ethyl acetate, methylethylke-

tone, butyl carbitol, cyclohexanone, triethylene glycol monobutyl ether, 1,2-hexanediol, propylene glycol monomethyl ether, isopropanol, methanol, water, isobornyl acrylate, 1,6-hexane diacrylate, and polyethylene glycol diacrylate; preferably a substance having strong surface activity to at least one kind of solvent from hexane, toluene, propylene glycol monomethyl ether, isobornyl acrylate, 1,6-hexanediacrylate, and polyethylene glycol diacrylate, more preferably a substance having a strong surface activity to at least one solvent selected from propylene glycol monomethyl ether, isobornyl acrylate, 1,6-hexane diacrylate, and polyethylene glycol diacrylate; and particularly preferably a substance having strong surface activity to at least one solvent selected from isobornyl acrylate, 1,6-hexane diacrylate, and polyethylene glycol diacrylate.

Whether a compound has strong surface activity to the solvents listed above can be determined by the procedures as described below.

#### (Procedures)

One solvent is selected from the solvents listed above and measure the surface tension thereof  $\gamma_{solvent}(0)$ . Add the objective compound in the same solvent used to measure the  $\gamma_{solvent}(0)$ , increase the concentration of the compound by the increment of 0.01% by mass, and measure the surface tension of the solution  $\gamma_{solvent}$  (saturated) at the point when the change in the surface tension with respect to the change in the concentration of the compound becomes 0.01 mN/m or less.

If the relationship between the  $\gamma_{solvent}(0)$  and the  $\gamma_{solvent}$  (saturated) satisfies the following relation, the compound can be determined to have strong surface activity to the solvent:

$$\gamma_{solvent}(0) - \gamma_{solvent}(\text{saturated}) > 1 \text{ (mN/m).}$$

Specific examples of the surfactants contained in the undercoating liquid include anionic surfactants such as dialkylsulfosuccinates, alkylnaphthalensulfonates and fatty acid salts; nonionic surfactants such as polyoxyethylenealkyl ethers, polyoxyethylenealkylallyl ethers, acetylene glycols and polyoxyethylene-polyoxypropylene block copolymers; cationic surfactants such as alkylamine salts and quaternary ammonium salts; and fluorine-based surfactants. Examples of other surfactants include the surfactants described in JP-A No. 62-173463 and JP-A No. 62-183457.

#### -Recording Medium

Any recording medium of permeable, non-permeable or slowly permeable can be used as the recording medium in the ink jet recording method in the invention. Among these, a non-permeable medium and a slowly permeable recording medium are preferable from the viewpoint that the effect of the invention can be remarkably displayed. The permeable recording medium refers to, for example, a recording medium having such properties that when a liquid droplet of 10 pL is dropped onto the recording medium, the permeation time for the total amount of the droplet is 100 ms or less. The description "substantially does not permeate" refers to, for example, the conditions where the permeability of the liquid droplets after the lapse of one minute is 5% or less. The slowly permeable recording medium refers to a recording medium having such properties that when a liquid droplet of 10 pL is dropped onto the recording medium, the permeating time for the total amount of the droplet is 100 ms or more.

Examples of the permeable recording media include plain paper, porous paper, and other recording media that are capable of absorbing a liquid.

Examples of the materials of the recording media which are non-permeable or slowly permeable include art paper, synthetic resin, rubber, resin coated paper, glass, metal, ceramic, and wood. In the invention, a composite recording

medium composed of some of the above materials in combination can also be used for the purpose of adding functions.

Any kind of synthetic resin can be used as the synthetic resin, and examples thereof include polyesters such as polyethylene terephthalate and polybutadiene terephthalate, polyolefins such as polyvinyl chloride, polystyrene, polyethylene, polyurethane, and polypropylene, acrylic resins, polycarbonate, acrylonitrile-butadiene-styrene copolymers, diacetate, triacetate, polyimide, cellophane, and celluloid. The thickness and shape of the recording medium when a synthetic resin is used are not particularly limited and the medium may be any shape of film, card and block, and may be either transparent or opaque.

As to the form of usage, the synthetic resin is preferably used in the form of a film for so-called light wrapping, and various non-absorbing plastics and a film thereof can be used. Examples of the plastic films include a PET film, an OPS film, an OPP film, a PNY film, a PVC film, a PE film, a TAC film, and a PP film. Examples of other plastics include polycarbonate resins, acrylic resins, ABS resins, polyacetal resins, PVA resins, and rubbers.

Examples of the resin coated papers include a transparent polyester film, an opaque polyester film, an opaque polyolefin resin film, and a paper supporting body having both sides laminated with a polyolefin resin. A paper supporting body having both sides laminated with a polyolefin resin is particularly preferable.

The kind of the metals is not particularly limited and preferable examples thereof include aluminum, iron, gold, silver, copper, nickel, titanium, chromium, molybdenum, silicon, lead, zinc, stainless steel, and composite materials thereof.

Further, ink jet recording can be performed on the label side of read-only optical disks such as CD-ROMs and DVD-ROMs, write-once optical disks such as CD-Rs and DVD-Rs, rewritable optical disks and the like.

#### -Ink and Undercoating Liquid-

The ink and the undercoating liquid used in the ink jet recording method in the invention will be explained in detail.

The ink is composed so as to at least form an image. The ink preferably contains at least one polymerizable or crosslinkable material, and further a polymerization initiator, a lipophilic solvent, a coloring agent, and other components depending on necessity.

The undercoating liquid preferably contains at least an oligomer and has a different composition from that of the ink. The undercoating liquid preferably contains at least one polymerizable or crosslinkable material, and may contain a polymerization initiator, a lipophilic solvent, a coloring agent, and other components depending on necessity.

The polymerization initiator is preferably capable of initiating a polymerization reaction or a crosslinking reaction with actinic energy rays. By using the polymerization initiator, the undercoating liquid applied onto the recording medium can be cured by irradiation with actinic energy rays.

Further, the undercoating liquid preferably contains a radical polymerizable composition. The radical polymerizable composition in the invention contains at least one radical polymerizable material and at least one radical polymerization initiator. By using the radical polymerizable composition, the curing reaction of the undercoating liquid can be performed with high sensitivity in a short time.

The ink in the invention is preferably contains a coloring agent. The undercoating liquid to be used in combination with such an ink preferably contains no coloring agent; contains a coloring agent to the amount of less than 1% by mass; or contains a white pigment as a coloring agent. Each component that constitutes each liquid will be described in detail.

#### (Oligomer)

The undercoating liquid of the invention includes at least one oligomer. By including an oligomer in the undercoating liquid, prevention of spreading of the ink ejected onto the partially cured undercoating liquid can be moderated so as to allow the ink to spread to some extent. Therefore, the dots formed by ejection spread to some extent, but not flatly, so that the shapes thereof are retained when the dots spread to connect with each other. For example, in a case where the dot density is low, generation of white spots can be prevented and a high degree of density can be obtained to details, due to the connection among the dots.

The oligomer is a polymer composed of a finite number (generally, from 5 to 100) of monomers connected to each other, which may be appropriately selected from known compounds called oligomers. In the invention, oligomers with a weight average molecular weight of from 400 to 10,000 (more preferably from 500 to 5,000) are preferably selected.

The oligomer in the invention may be of any kind, and examples thereof include olefin type oligomers (such as ethylene oligomers, propylene oligomers and butene oligomers), vinyl type oligomers (such as styrene oligomers, vinyl alcohol oligomers, vinyl pyrrolidone oligomers, acrylate oligomers and methacrylate oligomers), diene oligomers (such as butadiene oligomers, chloroprene rubbers and pentadiene oligomers), ring-opening polymerization type oligomers (such as di-, tri-, tetraethylene glycols, polyethylene glycols and polyethylimines), and polyaddition type oligomers (such as phenol resins, amino resins, xylene resins and ketone resins). Among these, oligoester acrylates are preferable, oligomers of urethane acrylate type, polyester acrylate type and epoxy acrylate type are more preferable, and oligomers of urethane acrylate type are most preferable.

Examples of the urethane acrylate type oligomers include oligomers of aliphatic urethane acrylate type and aromatic urethane acrylate type. Details of such oligomers are described in, for example, "Oligomer Handbook", edited by Junji Yoshikawa, The Chemical Daily Co., Ltd.

Examples of the commercially available urethane acrylate type oligomers include R1204, R1211, R1213, R1217, R1218, R1301, R1302, 1303, R1304, R1306, R1308, R1901 and R1150 (manufactured by DAI-ICHI KOGYO SEIYAKU CO., LTD.); Ebecryl Series such as Ebecryl 230, 270, 4858, 8402, 8804, 8807, 8803, 9260, 1290, 1290K, 5129, 4842, 8210, 210, 4827, 6700, 4450 and 220 (manufactured by DAICEL-CYTEC Company LTD.); NK OLIGO U-4HA, U-6HA, U-15HA, U-108A and U-200AX (manufactured by SHIN-NAKAMURA CHEMICAL CO., LTD.); and ARONIX M-1100, M-1200, M-1210, M-1310, M-1600 and M-1960 (manufactured by TOAGOSEI CO., LTD.).

Examples of the commercially available polyester acrylate type oligomers include Ebecryl Series such as Ebecryl 1770, IR467, 81, 84, 83, 80, 675, 800, 810, 812, 1657, 1810, IRR302, 450, 670, 830, 870, 1830, 1870, 2870, IRR267, 813, 55 IRR483 and 811 (manufactured by DAICEL-CYTEC Company LTD.); and ARONIX M-6100, M-6200, M-6250, M-6500, M-7100, M-8030, M-8060, M-8100, M-8530, M-8560 and M-9050 (manufactured by TOAGOSEI CO., LTD.).

Examples of the commercially available epoxy acrylate type oligomers include Ebecryl Series such as Ebecryl 600, 860, 2958, 3411, 3600, 3605, 3700, 3701, 3703, 3702, 3708, RDX63182 and 6040 (manufactured by DAICEL-CYTEC Company LTD.).

Among the oligomers, urethane acrylate oligomers are preferable from the viewpoint of imparting dot connecting properties.

The oligomer can be used alone or in combination of two or more kinds.

The content of the oligomer in the undercoating liquid is preferably from 5 to 50% by mass and more preferably from 10 to 40% by mass, with respect to the total mass of the undercoating liquid. When the content of the oligomer is within the above range, the state of spreading or connection of the dots of the ejected ink can be effectively secured, while suppressing the spreading of the dots to such an extent that the dot shape is maintained and image disorder or bleeding is not caused.

(Polymerizable or Crosslinkable Material)

The polymerizable or crosslinkable material in the invention causes polymerization or crosslinking by the action of an initiating species such as a radical generated from a polymerization initiator described later, or the like, and has a function to cure a composition containing the initiating species.

Known polymerizable or crosslinkable materials that cause a polymerization or crosslinking reaction such as a radical polymerization reaction or dimerization reaction can be applied as the polymerizable or crosslinkable material. Examples of the polymerizable or crosslinkable materials include an addition polymerizable compound having at least one ethylenically unsaturated double bond, a polymer compound having a maleimide group in a side chain, and a polymer having a group having an unsaturated double bond positioned adjacent to an aromatic core and is capable of photodimerization, such as a cinnamyl group, a cinnamylidene group, a chalcone group or the like, in a side chain. Among these, an addition polymerizable compound having at least one ethylenically unsaturated double bond is more preferable, and particularly preferably a compound selected from the compounds having at least one and more preferably two or more of terminal ethylenically unsaturated bonds (monofunctional or polyfunctional compound). It can be appropriately selected from the widely known compounds in the industrial field to which the invention is related, and examples thereof include a compound having a chemical form of a monomer, a prepolymer (i.e., a dimer, a trimer, and an oligomer), a mixture thereof, and a copolymer of these compounds.

The polymerizable or crosslinkable materials may be used alone, or in combination of two or more kinds.

The polymerizable or crosslinkable materials in the invention are particularly preferably various known radical polymerizable monomers that cause a polymerization reaction by an initiating species generated from a radical initiator.

Examples of the radical polymerization monomers include (meth)acrylates, (meth)acrylamides, aromatic vinyls, vinyl ethers, and compounds having an inner double bond (maleic acid, etc.). In this case, “(meth)acrylate” refers to both or either one of “acrylate” and “methacrylate,” and “(meth)acryl” refers to both or either one of “acryl” and “methacryl.”

Specific examples of the (meth)acrylates include the following compounds.

Specific examples of the monofunctional (meth)acrylates include hexyl (meth)acrylate, 2-ethylhexyl(meth)acrylate, tert-octyl(meth)acrylate, isoamyl (meth)acrylate, decyl (meth)acrylate, isodecyl(meth)acrylate, stearyl(meth)acrylate, isostearyl(meth)acrylate, cyclohexyl(meth)acrylate, 4-n-butylcyclohexyl(meth)acrylate, bornyl(meth)acrylate, isobornyl(meth)acrylate, benzyl(meth)acrylate, 2-ethylhexyl diglycol (meth)acrylate, butoxyethyl(meth)acrylate, 2-chloroethyl(meth)acrylate, 4-bromobutyl (meth)acrylate, cyanoethyl(meth)acrylate, benzyl(meth)acrylate, butoxymethyl (meth)acrylate, 3-methoxybutyl(meth)acrylate, alkoxyethyl(meth)acrylate, alkoxyethyl (meth)acrylate, 2-(2-methoxyethoxy)ethyl(meth)acrylate, 2-(2-butoxyethoxy)ethyl (meth)

acrylate, 2,2,2-trifluoroethyl(meth)acrylate, 1H, 1H,2H-perfluorodecyl (meth)acrylate, 4-butylphenyl(meth)acrylate, phenyl(meth)acrylate, 2,3,5,6-tetramethylphenyl(meth)acrylate, 4-chlorophenyl(meth)acrylate, phenoxyethyl (meth)acrylate, phenoxyethyl(meth)acrylate, glycidyl(meth)acrylate, glycidyloxybutyl (meth)acrylate, glycidyloxyethyl (meth)acrylate, glycidyloxypropyl(meth)acrylate, tetrahydrofurfuryl(meth)acrylate, hydroxalkyl(meth)acrylate, 2-hydroxyethyl (meth)acrylate, 3-hydroxypropyl(meth)acrylate,

2-hydroxypropyl(meth)acrylate, 2-hydroxybutyl(meth)acrylate, 4-hydroxybutyl (meth)acrylate, dimethylaminoethyl(meth)acrylate, diethylaminoethyl(meth)acrylate, dimethyaminopropyl(meth)acrylate, diethylaminopropyl(meth)acrylate, trimethoxysilylpropyl(meth)acrylate, trimethylsilylpropyl(meth)acrylate, polyethyleneoxide monomethylether (meth)acrylate, oligoethyleneoxide monomethylether (meth)acrylate, polyethyleneoxide (meth)acrylate, oligoethyleneoxide monoalkylether (meth)acrylate, polyethyleneoxide monoalkylether (meth)acrylate, dipropylene glycol (meth)acrylate, polypropyleneoxide monoalkylether (meth)acrylate, oligopropyleneoxide monoalkylether (meth)acrylate, 2-methacryloyloxyethyl succinic acid, 2-methacryloyloxyhexahydrophthalic acid, 2-methacryloyloxyethyl-2-hydroxypropyl phthalate, butoxydiethylene glycol (meth)acrylate, trifluoroethyl(meth)acrylate, perfluoroctylethyl(meth)acrylate, 2-hydroxy-3-phenoxypropyl(meth)acrylate, EO-modified phenol (meth)acrylate, EO-modified cresol (meth)acrylate, EO-modified nonylphenol (meth)acrylate, PO-modified nonylphenol (meth)acrylate, and EO-modified-2-ethylhexyl (meth)acrylate.

Specific examples of the bifunctional (meth)acrylates include 1,6-hexadiol di(meth)acrylate, 1,10-decanediol di(meth)acrylate, neopentyl glycol di(meth)acrylate, 2,4-dimethyl-1,5-pentanediol di(meth)acrylate, butylethylpropanediol (meth)acrylate, ethoxylated cyclohexanemethanol di(meth)acrylate, polyethylene glycol di(meth)acrylate, oligoethylene glycol di(meth)acrylate, ethylene glycol di(meth)acrylate, 2-ethyl-2-butyl-butanediol di(meth)acrylate, hydroxypivalic neopentyl glycol di(meth)acrylate, EO-modified bisphenol A di(meth)acrylate, bisphenol F polyethoxy di(meth)acrylate, polypropylene glycol di(meth)acrylate, oligopropylene glycol di(meth)acrylate, 1,4-butanediol di(meth)acrylate, 2-ethyl-2-butylpropanediol di(meth)acrylate, 1,9-nonane di(meth)acrylate, propoxylated ethoxylated bisphenol A di(meth)acrylate, and tricyclodecane di(meth)acrylate.

Specific examples of the trifunctional (meth)acrylates include trimethylolpropane tri(meth)acrylate, trimethylolethane tri(meth)acrylate, alkyleneoxide-modified tri(meth)acrylate of trimethylolpropane, pentaerythritol tri(meth)acrylate, dipentaerythritol tri(meth)acrylate, trimethylolpropane tris((meth)acryloyloxypropyl)ether, isocyanuric alkyleneoxide-modified tri(meth)acrylate, propionic dipentaerythritol tri(meth)acrylate, tris((meth)acryloyloxyethyl)isocyanurate, hydroxypivalaldehyde-modified dimethylolpropane tri(meth)acrylate, sorbitol tri(meth)acrylate, propoxylated trimethylolpropane tri(meth)acrylate, and ethoxylated glycerin triacrylate.

Specific examples of the tetrafunctional (meth)acrylates include pentaerythritol tetra(meth)acrylate, sorbitol tetra(meth)acrylate, ditrimethylolpropane tetra(meth)acrylate, propionic dipentaerythritol tetra(meth)acrylate, and ethoxylated pentaerythritol tetra(meth)acrylate.

Specific examples of the pentafunctional (meth)acrylates include sorbitol penta(meth)acrylate and dipentaerythritol penta(meth)acrylate.

Specific examples of the hexafunctional (meth)acrylates include dipentaerythritol hexa(meth)acrylate, sorbitol hexa(meth)acrylate, alkyleneoxide-modified hexa(meth)acrylate of phosphazene, and caprolactone-modified dipentaerythritol hexa(meth)acrylate.

Examples of the (meth)acrylamides include (meth)acrylamide, N-methyl(meth)acrylamide, N-ethyl(meth)acrylamide, N-propyl(meth)acrylamide, N-n-butyl(meth)acrylamide, N-t-butyl(meth)acrylamide, N-butoxymethyl(meth)acrylamide, N-isopropyl(meth)acrylamide, N-methylol(meth)acrylamide, N,N-dimethyl(meth)acrylamide, N,N-diethyl(meth)acrylamide, and (meth)acryloylmorpholine.

Specific examples of the aromatic vinyls include styrene, methylstyrene, dimethylstyrene, trimethylstyrene, ethylstyrene, isopropylstyrene, chloromethylstyrene, methoxystyrene, acetoxystyrene, chlorstyrene, dichlorstyrene, bromstyrene, methyl vinylbenzoate, 3-methylstyrene, 4-methylstyrene, 3-ethylstyrene, 4-ethylstyrene, 3-propylstyrene, 4-propylstyrene, 3-butylstyrene, 4-butylstyrene, 3-hexylstyrene, 4-hexylstyrene, 3-octylstyrene, 4-octylstyrene, 3-(2-ethylhexyl)styrene, 4-(2-ethylhexyl)styrene, allylstyrene, isopropenylstyrene, butenylstyrene, octenylstyrene, 4-t-butoxycarbonylstyrene, 4-methoxystyrene, and 4-t-butoxystyrene.

Specific examples of the vinylethers include the following compounds.

Specific examples of the monofunctional vinylethers include methylvinylether, ethylvinylether, propylvinylether, n-butylvinylether, t-butylvinylether, 2-ethylhexylvinylether, n-nonylvinylether, laurylvinylether, cyclohexylvinylether, cyclohexylmethylvinylether, 4-methylcyclohexylmethylvinylether, benzylvinylether, dicyclopentenylvinylether, 2-dicyclopentenoxyethylvinylether, methoxyethylvinylether, ethoxyethylvinylether, butoxyethylvinylether, methoxyethoxyethylvinylether, ethoxyethoxyethylvinylether, methoxypolyethylene glycol vinylether, tetrahydrofurfurylvinylether, 2-hydroxyethylvinylether, 2-hydroxypropylvinylether, 4-hydroxybutylvinylether, 4-hydroxymethylcyclohexylmethylvinylether, diethylene glycol monovinylether, polyethylene glycol vinylether, chlorehylvinylether, chlorbutylvinylether, chlorethoxyethylvinylether, phenylethylvinylether, and phenoxypropylethylene glycol vinylether.

Examples of the polyfunctional vinylethers include divinylethers such as ethylene glycol divinylether, diethylene glycol divinylether, polyethylene glycol divinylether, propylene glycol divinylether, butylene glycol divinylether, hexanediol divinylether, bisphenol A alkyleneoxide divinylether and bisphenol F alkyleneoxide divinylether; and polyfunctional vinylethers such as trimethylethane trivinylether, trimethylolpropane trivinylether, trimethylolpropane tetravinylether, glycerin trivinylether, pentaerythritol tetravinylether, dipentaerythritol pentavinylether, dipentaerythritol hexavinylether, ethyleneoxide added trimethylolpropane trivinylether, propyleneoxide added trimethylolpropane trivinylether, ethyleneoxide added trimethylolpropane tetravinylether, propyleneoxide added trimethylolpropane tetravinylether, ethyleneoxide added pentaerythritol tetravinylether, propyleneoxide added pentaerythritol tetravinylether, ethyleneoxide added dipentaerythritol hexavinylether, and propyleneoxide added dipentaerythritol hexavinylether.

The vinylether compound is preferably a di- or tri-vinylether compound from the viewpoint of curing property,

adhesion to a recording medium, surface hardness of the formed image or the like, and particularly preferably a divinylether compound.

Other examples of the radical polymerizable monomers in the invention include vinylesters such as vinyl acetate, vinyl propionate and vinyl versatate; allylestes such as allyl acetate; halogen-containing monomers such as vinylidene chloride and vinyl chloride; cyanide vinyls such as (meth)acrylonitrile; and olefins such as ethylene and propylene.

Among the above, the radical polymerizable monomer is preferably a (meth)acrylate and (meth)acrylamides in view of curing speed, and particularly preferably a (meth)acrylate of tetrafunctional or more in view of curing speed. From the viewpoint of the viscosity of the ink composition, it is preferable to use a polyfunctional (meth)acrylate in combination with a monofunctional or bifunctional (meth)acrylate or (meth)acrylamide.

The content of the polymerizable or crosslinkable material in the ink and the undercoating liquid is preferably in the range of from 50 to 99.6% by mass with respect to the total solid content (mass) in each liquid droplet, more preferably in the range of from 70 to 99.0% by mass, and further preferably in the range of from 80 to 99.0% by mass.

The content of the polymerizable or crosslinkable material in the liquid droplet is preferably in the range of from 20 to 98% by mass with respect to the total mass of each liquid droplet, more preferably in the range of from 40 to 95% by mass, and particularly preferably in the range of from 50 to 90% by mass.

(Polymerization Initiator)

The ink and the undercoating liquid can be preferably composed using at least one polymerization initiator, and it is preferable that at least the undercoating liquid contains the polymerization initiator. This polymerization initiator is a compound that generates an initiating species such as a radical with the application of energy such as active light, heat, or both of these, and initiates and promotes the polymerization or crosslinking reaction of the above-described polymerizable or crosslinkable materials, thereby curing the undercoating liquid or the ink.

From the aspect of the polymerizability, the polymerization initiator preferably is the one that causes a radical polymerization, and is particularly preferably a photopolymerization initiator.

The photopolymerization initiator is a compound that causes a chemical change by the action of light and an interaction with a sensitizing dye in an electronically excited state and produces at least any one of a radical, acid and base, and a photoradical generator is preferable from the viewpoint that the polymerization can be initiated with a simple means as exposure.

The photopolymerization initiator in the invention can be selected from the photopolymerization initiators having sensitivity to active light rays such as ultraviolet rays of from 400 to 200 nm, far ultraviolet rays, g-rays, h-rays, i-rays, KrF excimer laser beams, ArF excimer laser beams, electron beams, X-rays, molecular beams or ion beams.

Specifically, known photopolymerization initiators in the art can be used without limitation, such as the ones described in Bruce M. Monroe et al., *Chemical Reviews*, 93, 435 (1993); R. S. Davidson, *Journal of Photochemistry and Biology A: Chemistry*, 73, 81 (1993); J. P. Faussier, "Photoinitiated Polymerization—Theory and Applications", *Rapra Review Report*, vol. 9, Rapra Technology (1998); and M. Tsunooka et al., *Prog Polym. Sci.*, 21, 1 (1996). Further, a group of compounds that oxidatively or reductively generates a bond cleavage through interaction with a sensitizing dye in an electroni-

cally excited state as described in F. D. Saeva, *Topics in Current Chemistry*, 156, 59 (1990); G. G. Maslak, *Topics in Current Chemistry*, 168, 1 (1993); H. B. Shuster et al., *JACS*, 112, 6329 (1990); I. D. F. Eaton et al., *JACS*, 102, 3298 (1980), and the like.

Preferable photopolymerization initiators can be exemplified by: (a) aromatic ketones; (b) aromatic onium salt compounds; (c) organic peroxides; (d) hexaaryliimidazoles compounds; (e) ketoxime ester compounds; (f) borate compounds; (g) azinium compounds; (h) metallocene compounds; (i) active ester compounds; and (j) compounds having a carbon-halogen bond.

Preferable examples of the (a) aromatic ketones include a compound having a benzophenone skeleton or a thioxanthone skeleton described in J. P. Fouassier, J. F. Rabek, "Radiation Curing in Polymer Science and Technology", pp. 77-117 (1993). More preferable examples of the (a) aromatic ketones include  $\alpha$ -thiobenzophenone compounds described in Japanese Patent Publication (JP-B) No. 47-6416, benzoin ether compounds described in JP-B No. 47-3981,  $\alpha$ -substituted benzoin compounds described in JP-B No. 47-22326, benzoin derivatives described in JP-B No. 47-23664, arylphosphonic esters described in JP-A No. 57-30704, dialkoxybenzophenone described in JP-B No. 60-26483, benzoinethers described in JP-B No. 60-26403 and JP-B No. 62-81345,  $\alpha$ -aminobenzophenones described in JP-B No. 1-34242, U.S. Pat. No. 4,318,791 and EP No. 0284561A1, p-di(dimethylaminozenzoyl)benzene described in JP-A No. 2-211452, thio-substituted aromatic ketones described in JP-A No. 61-194062, acylphosphine sulfides described in JP-B No. 2-9597, acylphosphines described in JP-B No. 2-9596, thioxanthones described in JP-B No. 63-61950, and coumarins described in JP-B No. 59-42864.

Examples of the (b) aromatic onium salt compounds include aromatic onium salts of the elements in the groups of V, VI, and VII in the periodic table, specifically N, P, As, Sb, Bi, O, S, Se, Te or I. Preferable examples thereof include iodonium salts described in EP No. 104143, U.S. Pat. No. 4,837,124, JP-A No. 2-150848 and JP-A No. 2-96514; sulphonium salts described in EP Nos. 370693, 233567, 297443, 297442, 279210 and 422570, U.S. Pat. Nos. 3,902,144, 4,933,377, 4,760,013, 473-4444 and 2833827; diazonium salts (such as benzene diazonium that may have a substituent); diazonium salt resins (such as formaldehyde resins of diazophenylamine); N-alkoxypyridium salts (examples thereof include compounds described in U.S. Pat. No. 4,743, 528, JP-A Nos. 63-138345, 63-142345, 63-142346 and JP-B No. 46-42363; and specific examples thereof include 1-methoxy-4-phenylpyridium and tetrafluoroborate), and compounds described in JP-B Nos. 52-147277, 52-14278 and 52-14279. Radicals and acids are produced as the active species.

Examples of the (c) "organic peroxides" includes almost all of the organic compounds having one or more oxygen-oxygen bonds in the molecule and can be exemplified by ester peroxide type compounds such as

3,3',4,4'-tetrakis(t-butylperoxycarbonyl)benzophenone, 3,3',4,4'-tetrakis(t-amylperoxycarbonyl)benzophenone, 3,3',4,4'-tetrakis(t-hexylperoxycarbonyl)benzophenone, 3,3',4,4'-tetrakis(t-octylperoxycarbonyl)benzophenone, 3,3',4,4'-tetrakis(cumylperoxycarbonyl)benzophenone, 3,3',4,4'-tetrakis(p-isopropylcumylperoxycarbonyl)benzophenone, and di-t-butylperoxyisophthalate.

Examples of the (d) hexaaryliimidazoles include the lophin dimers described in JP-B Nos. 45-37377 and 44-86516 such as

2,2'-bis(o-chlorophenyl)-4,4',5,5'-tetraphenylbiimidazole, 2,2'-bis(o-bromophenyl)-4,4',5,5'-tetraphenylbiimidazole, 2,2'-bis(o,p-dichlorophenyl)-4,4',5,5'-tetraphenylbiimidazole, 2,2'-bis(o-chlorophenyl)-4,4',5,5'-tetrakis(m-methoxyphenyl)biimidazole, 2,2'-bis(o,o'-dichlorophenyl)-4,4',5,5'-tetraphenylbiimidazole, 2,2'-bis(o-nitrophenyl)-4,4',5,5'-tetraphenylbiimidazole, 2,2'-bis(o-methylphenyl)-4,4',5,5'-tetraphenylbiimidazole, and 2,2'-bis(o-trifluorophenyl)-4,4',5,5'-tetraphenylbiimidazole.

Examples of the (e) ketoxime esters include 3-benzoyloxyiminobutane-2-one, 3-acetoxymonobutane-2-one, 3-propionyloxyiminobutane-2-one,

2-acetoxyminopentane-3-one, 2-acetoxymino-1-phenylpropane-1-one, 2-benzoyloxyimino-1-phenylpropane-1-one, 3-p-toluenesulfonyloxyimino-1-phenylpropane-2-one, and 2-ethoxycarbonyloxyimino-1-phenylpropane-1-one.

Examples of the (f) borate compounds include the compounds described in U.S. Pat. Nos. 3,567,453 and 4,343,891, and EP Nos. 109,772 and 109,773.

Examples of the (g) azinium compounds are include the compounds having a N—O bond described in JP-A Nos. 63-138345, 63-142345, No. 63-142346 and 63-143537, and JP-B No. 46-42363.

Examples of the (h) metallocene compounds include the titanocene compounds described in JP-A Nos. 59-152396, 61-151197, 63-41484, 2-249, and 2-4705; and the iron-arene complexes described in JP-A Nos. 1-304453 and 1-152109.

Specific examples of the titanocene compounds include di-cyclopentadienyl-Ti-di-chloride, di-cyclopentadienyl-Ti-bis-phenyl, di-cyclopentadienyl-Ti-bis-2,3,4,5,6-pentafluorophenyl-1-yl, di-cyclopentadienyl-Ti-bis-2,3,5,6-tetrafluorophenyl-1-yl, di-cyclopentadienyl-Ti-bis-2,4,6-trifluorophenyl-1-yl, di-cyclopentadienyl-Ti-2,6-difluorophenyl-1-yl, di-cyclopentadienyl-Ti-bis-2,4-difluorophenyl-1-yl, di-methylcyclopentadienyl-Ti-bis-2,3,4,5,6-pentafluorophenyl-1-yl, di-methylcyclopentadienyl-Ti-bis-2,3,5,6-tetrafluorophenyl-1-yl, di-methylcyclopentadienyl-Ti-bis-2,4-difluorophenyl-1-yl, bis(cyclopentadienyl)-bis(2,6-difluoro-3-(pyri-1-yl)phenyl) titanium, bis(cyclopentadienyl)bis[2,6-difluoro-3-(methylsulfoneamide)phenyl]titanium, and bis(cyclopentadienyl)bis[2,6-difluoro-3-(N-butyliaroyl-amino)phenyl]titanium.

Examples of the (i) active ester compounds include the nitrobenzylester compounds described in EP Nos. 0290750, 046083, 156153, 271851 and 0388343, USP Nos. 3901710 and 4181531, JP-A Nos. 60-198538 and 53-133022; imino-sulfonate compounds described in EP Nos. 0199672, 84515, 044115 and 0101122, U.S. Pat. Nos. 4,618,564, 4,371,605 and 4431774, JP-A Nos. 64-18143, 2-245756 and 4-365048; and the compounds described in JP-B No. 62-6223, JP-B No. 63-14340, and JP-A No. 59-174831.

Preferable examples of the (j) compounds having a carbon-halogen bond include the compounds described in Wakabayashi et al., *Bull. Chem. Soc. Japan*, 42, 2924 (1969), compounds described in U.K. Patent No. 1388492, compounds

described in JP-A No. 53-133428, and the compounds described in German Patent No. 3337024.

Further, preferable examples of the compounds also include the compounds described in F. C. Schaefer et al., *J. Org. Chem.*, 29, 1527 (1964), compounds described in JP-A Nos. 62-58241 and 5-281728, compounds described in German Patent Nos. 2641100 and 3333450, and the compounds described in German Patent Nos. 3021590 and 3021599.

Examples of the photopolymerization initiator in the invention may be the compounds as shown below, but are not limited thereto. In the following formulae, Ar represents an aromatic group.



-continued



**27**

-continued

**28**

-continued



**29**

-continued

**30**

-continued



31



The polymerization initiator preferably has a high degree of sensitivity. However, from the viewpoint of storage stability, the polymerization initiator that does not cause thermal decomposition at a temperature up to 80° C. is preferably selected.

The polymerization initiator may be used alone or in combination of two or more kinds. Known sensitizers may be also used in combination for the purpose of improving the sensitivity as long as the effect of invention is not spoiled.

The content of the polymerization initiator in the undercoating liquid is preferably in the range of from 0.5 to 20% by mass with respect to the amount of the polymerizable material contained in the undercoating liquid, more preferably from 1 to 15% by mass, and particularly preferably from 3 to 10% by mass, from the viewpoint of temporal stability, curing property and curing speed. By containing the polymerization initiator of the amount in the above-described range, occurrence of precipitation or separation with the lapse of time and deterioration in the performances such as ink strength or rubbing resistance after curing can be suppressed.

The polymerization initiator may be contained in the ink as well as in the undercoating liquid, and the content thereof can be appropriately determined in the range where the storage stability of the ink can be maintained at the desired level. The content of the polymerization initiator in the ink droplet is preferably from 0.5 to 20% by mass with respect to the polymerizable or crosslinkable compound in the ink, and more preferably from 1 to 15% by mass.

#### (Sensitizing Dye)

A sensitizing dye may be added for the purpose of improving the sensitivity of the photopolymerization initiator in the invention. Preferred examples of the sensitizing dyes are the compounds included in the following compounds below and have an absorption wavelength in the range of from 350 nm to 450 nm.

Polynuclear aromatics (for example, pyrene, perylene, and triphenylene), xanthenes (for example, fluorescein, eosin, erythrosine, rhodamine B, and rose bengal), cyanines (for example, thiacyanocyanine and oxacyanocyanine), merocyanines (for example, merocyanine and carbomerocyanine), thiazines (for example, thionine, methylene blue, and toluyzine blue), acridines (for example, acridine orange, chloroflavin, and acriflavin), anthraquinones (for example, anthraquinone), squaryliums (for example, squarylium), and cumarins (for example, 7-diethylamino-4-methylcumarin).

Examples of the preferred sensitizing dyes are the compounds represented by the following Formulas (IX) to (XIII).

32



In Formula (IX),  $A^1$  represents a sulfur atom or  $—NR^{50}—$ ,  $R^{50}$  represents an alkyl group or an aryl group,  $L^2$  represents a non-metal atomic group that forms a basic nucleus of a dye together with the adjacent  $A^1$  and the adjacent carbon atom,  $R^{51}$  and  $R^{52}$  each independently represent a hydrogen atom or a monovalent non-metal atomic group, wherein  $R^{51}$  and  $R^{52}$  may form an acid nucleus of a dye by bonding to each other.  $W$  represents an oxygen atom or a sulfur atom.

In Formula (X),  $Ar^1$  and  $Ar^2$  each independently represent an aryl group, and connect with each other via a bond by  $-L^3-$ , wherein  $L^3$  represents  $—O—$  or  $—S—$ .  $W$  represents an oxygen atom or a sulfur atom.

In Formula (XI),  $A^2$  represents a sulfur atom or  $—NR^{59}—$ ,  $L^4$  represents a non-metal atomic group that forms a basic nucleus of a dye together with the adjacent  $A^2$  and the carbon atom.  $R^{53}$ ,  $R^{54}$ ,  $R^{55}$ ,  $R^{56}$ ,  $R^{57}$ , and  $R^{58}$  each independently represent a group of a monovalent non-metal atomic group, and  $R^{59}$  represents an alkyl group or an aryl group.

In Formula (XII),  $A^3$  and  $A^4$  each independently represent  $—S—$ ,  $NR^{62}$ , or  $—NR^{63}$ ,  $R^{62}$  and  $R^{63}$  each independently represent a substituted or unsubstituted alkyl group or a substituted or unsubstituted aryl group,  $L^5$  and  $L^6$  each independently represent a non-metal atomic group that forms a basic nucleus of a dye together with the adjacent  $A^3$ ,  $A^4$ , and the adjacent carbon atom, and  $R^{60}$  and  $R^{61}$  each independently represent a hydrogen atom or a monovalent non-metal atomic group, or can form an aliphatic or aromatic ring by bonding to each other.

In Formula (XIII),  $R^{66}$  represents an aromatic ring or a hetero ring that may have a substituent, and  $A^5$  represents an oxygen atom, a sulfur atom, or  $—NR^{67}—$ .  $R^{64}$ ,  $R^{65}$ , and  $R^{67}$  each independently represent a hydrogen atom or a monovalent

**33**

lent non-metal atomic group, and R<sup>67</sup> and R<sup>64</sup>, and R<sup>65</sup> and R<sup>67</sup> can bond to each other to form an aliphatic or an aromatic ring.

Specific examples of the compounds represented with the Formulas (IX) to (XIII) include Exemplified Compounds (A-1) to (A-20) shown as follows.



(A-1) 10



(A-2) 20



(A-3)



(A-4)



(A-5)



(A-6)

**34**

-continued

(A-7)



(A-8)



(A-9)



(A-10)



(A-11)



(A-12)



(A-13)



(A-14)

35

-continued



(A-15)



(A-16)



(A-17)



(A-18)



(A-19)



(A-20)

## (Cosensitizer)

Known compounds having the capacity to further improve sensitivity or suppress the inhibition of polymerization by oxygen may be added as a cosensitizer.

Examples of the cosensitizers include amines such as the compounds described in M. R. Sander et al., *Journal of Polymer Society*, vol. 10, 3173 (1972), JP-B No. 44-20189, JP-A Nos. 51-82102, 52-134692, 59-138205, 60-84305, 62-18537 and 64-33104, and Research Disclosure No. 33825. Specific compounds thereof include triethanolamine, p-dimethylaminobenzenethylester, p-formyldimethylaniline, and p-methylthiodimethylaniline.

Other examples of the cosensitizers include thiols and sulfides such as the thiol compounds described in JP-A No. 53-702, JP-B No. 55-500806, and JP-A No. 5-142772, and the disulfide compounds described in JP-A No. 56-75643. Specific examples thereof include 2-mercaptopbenzothiazole, 2-mercaptopbenzoxazole, 2-mercaptopbenzimidazole, 2-mercapto-4-(3H)-quinazoline, and  $\beta$ -mercaptopnaphthalene.

Other examples of the cosensitizers further include amino acid compounds (for example, N-phenylglycine), the organic

36

metal compounds described in JP-B No. 48-42965 (for example, tributyl tin acetate), the hydrogen donors described in JP-B No. 55-34414, the sulfur compounds described in JP-A No. 6-308727 (for example, trithiane), the phosphor compounds described in JP-A No. 6-250387 (for example, diethylphosphite), and the compounds of Si—H and Ge—H described in JP-A No. 8-65779. (Coloring Agent)

The ink and the undercoating liquid preferably contain at least one coloring agent, and more preferably a coloring agent is contained at least in the ink. The coloring agent may be included in the undercoating liquid and other liquids other than the ink.

The coloring agent is not particularly limited, and may be appropriately selected from known water-soluble dyes, oil-soluble dyes, and pigments. The ink and the undercoating liquid in the invention are preferably composed as a non-water soluble organic solvent system from the viewpoint of the effect of the invention, and oil-soluble dyes or pigments that readily dissolve and uniformly disperse in a non-water soluble medium are preferably used.

The content of the coloring agent in the ink is preferably from 1 to 30% by mass, more preferably from 1.5 to 25% by mass, and particularly preferably from 2 to 15% by mass. When the undercoating liquid contains a white pigment, the content thereof in the undercoating liquid is preferably from 2 to 45% by mass, and more preferably from 4 to 35% by mass.

## (Pigment)

Details of the pigments will be explained focusing on the preferable examples thereof in the invention.

In the invention, it is preferable that a pigment is used as the coloring agent. Either of organic pigments and inorganic pigments can be used as the pigment, but a carbon black pigment can be named as a preferable black pigment. The pigments of black and the three basic colors of cyan, magenta, and yellow are generally used, but pigments having other hues such as red, green, blue, brown and white, metallic-glossy pigments such as gold and silver, and body pigments of colorless or a light color can also be used depending on the purposes.

Examples of the organic pigments are not limited by the hues thereof, and include the pigments of perylene, perynone, quinacridone, quinacridone quinone, anthraquinone, anthanthrone, benzimidazolone, disazo condensation, disazo, azo, indanthrone, phthalocyanine, triarylcyanium, dioxazine, aminoanthraquinone, diketopyrrolopyrrole, thio indigo, isoindoline, isoindolinone, pyranthrone and isoviolanthrone, and mixtures thereof.

Further specific examples of the pigments include perylene-based pigments such as C. I. Pigment Red 190 (C. I. No. 71140), C. I. Pigment Red 224 (C. I. No. 71127), and C. I. Pigment Violet 29 (C. I. No. 71129); perynone-based pigments such as C. I. Pigment Orange 43 (C. I. No. 71105) and C. I. Pigment Red 194 (C. I. No. 71100); quinacridone-based pigments such as C. I. Pigment Violet 19 (C. I. No. 73900), C. I. Pigment Violet 42, C. I. Pigment Red 122 (C. I. No. 73915), C. I. Pigment Red 192, C. I. Pigment Red 202 (C. I. No. 73907), C. I. Pigment Red 207 (C. I. No. 73900 and No. 73906), and C. I. Pigment Red 209 (C. I. No. 73905); quinacridone quinone-based pigments such as C. I. Pigment Red 206 (C. I. No. 73900/73920), C. I. Pigment Orange 48 (C. I. No. 73900/73920), and C. I. Pigment Orange 49 (C. I. No. 73900/73920); anthraquinone-based pigments such as C. I. Pigment Yellow 147 (C. I. No. 60645); anthoanthrone-based pigments such as C. I. Pigment Red 168 (C. I. No. 59300); benzimidazolone-based pigments such as C. I. Pigment

Brown 25 (C. I. No. 12510), C. I. Pigment Violet 32 (C. I. No. 12517), C. I. Pigment Yellow 180 (C. I. No. 21290), C. I. Pigment Yellow 181 (C. I. No. 11777), C. I. Pigment Orange 62 (C. I. No. 11775), and C. I. Pigment Red 185 (C. I. No. 12516); disazo condensation-based pigments such as C. I. Pigment Yellow 93 (C. I. No. 20710), C. I. Pigment Yellow 94 (C. I. No. 20038), C. I. Pigment Yellow 95 (C. I. No. 20034), C. I. Pigment yellow 128 (C. I. No. 20037), C. I. Pigment Yellow 166 (C. I. No. 20035), C. I. Pigment Orange 34 (C. I. No. 21115), C. I. Pigment Orange 13 (C. I. No. 21110), C. I. Pigment Orange 31 (C. I. No. 20050), C. I. Pigment Red 144 (C. I. No. 20735), C. I. Pigment Red 166 (C. I. No. 20730), C. I. Pigment Red 220 (C. I. No. 20055), C. I. Pigment Red 221 (C. I. No. 20065), C. I. Pigment Red 242 (C. I. No. 20067), C. I. Pigment Red 248, C. I. Pigment Red 262, and C. I. Pigment Brown 23 (C. I. No. 20060);

Disazo-based pigments such as C. I. Pigment Yellow 13 (C. I. No. 21100), C. I. Pigment Yellow 83 (C. I. No. 21108), and C. I. Pigment Yellow 188 (C. I. No. 21094); azo-based pigments such as C. I. Pigment Red 187 (C. I. No. 12486), C. I. Pigment Red 170 (C. I. No. 12475), C. I. Pigment Yellow 74 (C. I. No. 11714), C. I. Pigment Yellow 150 (C. I. No. 48545), C. I. Pigment Red 48 (C. I. No. 15865), C. I. Pigment Red 53 (C. I. No. 15585), C. I. Pigment Orange 64 (C. I. No. 12760), and C. I. Pigment Red 247 (C. I. No. 15915); indanthrone-based pigments such as C. I. Pigment Blue 60 (C. I. No. 69800); phthalocyanine-based pigments such as C. I. Pigment Green 7 (C. I. No. 74260), C. I. Pigment Green 36 (C. I. No. 74265), C. I. Pigment Green 37 (C. I. No. 74255), C. I. Pigment Blue 16 (C. I. No. 74100), C. I. Pigment Blue 75 (C. I. No. 74160: 2), and 15 (C. I. No. 74160); triarylcarbonium-based pigments such as C. I. Pigment Blue 56 (C. I. No. 42800) and C. I. Pigment Blue 61 (C. I. No. 42765: 1); dioxadine-based pigments such as C. I. Pigment Violet 23 (C. I. No. 51319) and C. I. Pigment Violet 37 (C. I. No. 51345); aminoanthraquinone-based pigments such as C. I. Pigment Red 177 (C. I. No. 65300); diketopyrrolopyrrole-based pigments such as C. I. Pigment Red 254 (C. I. No. 56110), C. I. Pigment 255 (C. I. No. 561050), C. I. Pigment Red 264, C. I. Pigment Red 272 (C. I. No. 561150), C. I. Pigment Orange 71, and C. I. Pigment Orange 73; thio indigo-based pigments such as C. I. Pigment Red 88 (C. I. No. 73312); isoindoline-based pigments such as C. I. Pigment Yellow 139 (C. I. No. 56298) and C. I. Pigment Orange 66 (C. I. No. 48210); isoindolinone-based pigments such as C. I. Pigment Yellow 109 (C. I. No. 56284) and C. I. Pigment Orange 61 (C. I. No. 11295); pyranthrone-based pigments such as C. I. Pigment Orange 40 (C. I. No. 59700) and C. I. Pigment Red 216 (C. I. No. 59710); and isoviolanthrone-based pigments such as C. I. Pigment Violet 31 (60010).

In the invention, two or more kinds of the organic pigments or solid solutions of the organic pigments can be combined and used.

Other materials such as particles composed of a core of silica, alumina, resin or the like having a dye or a pigment fixed on the surface, an insoluble laked compound of a dye, colored emulsion and colored latex can also be used as the pigment. Further, a pigment coated with a resin can be also used, which is called a micro capsule pigment and the products thereof are commercially available from DAINIPPON INK AND CHEMICALS, INC., TOYO INK MFG CO., LTD. and the like.

The volume average particle diameter of the pigment particles contained in the liquid is preferably in the range of from 10 to 250 nm, from the viewpoint of the balance between optical concentration and storage stability, and further preferably from 50 to 200 nm. The volume average particle diam-

eter of the pigment particles can be measured with a particle diameter distribution analyzer such as LB-500 (manufactured by HORIBA, LTD.).

The coloring agents may be used alone or in the form of a mixture of two or more kinds thereof. Further, different coloring agents may be used in different liquid droplets to be ejected and liquids, or the same coloring agent may be used therein.

**(Other Components)**

Components other than the ones described above such as known additives can also be used as appropriate according to usage.

**<Storage Stabilizer>**

A storage stabilizer can be added in the ink and the under-coating liquid according to the invention (preferably in the ink) for the purpose of suppressing undesired polymerization during storage. The storage stabilizer is preferably used together with the polymerizable or crosslinkable material, and is preferably soluble in the liquid droplets or liquid or other coexistent components in which the storage stabilizer is contained.

Examples of the storage stabilizers include a quaternary ammonium salt, hydroxylamines, cyclic amides, nitrites, substituted ureas, heterocyclic compounds, organic acids, hydroquinone, hydroquinone monoethers, organic phosphines and copper compounds, and specific examples thereof include benzyltrimethylammonium chloride, diethylhydroxylamine, benzothiazole, 4-amino-2,2,6,6-tetramethylpiperazine, citric acid, hydroquinone monomethylether, hydroquinone monobutylether and copper naphthenate.

The addition amount of the storage stabilizer is preferably adjusted as appropriate according to the activity of the polymerization initiator, polymerization capability of the polymerizable or crosslinkable material, or the type of the storage stabilizer, but is preferably from 0.005 to 1% by mass in terms of the solid content, more preferably from 0.01 to 0.5% by mass, and further preferably 0.01 to 0.2% by mass, in view of the balance between storage stability and curing property.

**<Conductive Salt>**

Conductive salts are solid compounds that improve conductivity. In the invention, it is preferable that the conductive salt is not substantially used since there is a large possibility that they deposit at the time of storage, but appropriate amount thereof may be added when the solubility is in good condition by enhancing the solubility of the conductive salt or using a substance having high solubility in the liquid component, and the like.

Examples of the conductive salts include potassium thiocyanate, lithium nitrate, ammonium thiocyanate and dimethylamine hydrochloride.

**<Solvent>**

Known solvents can be used in the invention, as necessary. The solvent can be used for the purpose of improving the polarity, viscosity or the surface tension of the liquid (ink), improving the solubility or dispersibility of the coloring agent, adjusting the conductivity, or adjusting the printing performance.

The solvent in the invention is preferably a non-water soluble liquid that does not contain an aqueous solvent from the viewpoint of recording a high quality image that dries quickly and is uniform in line width, and is more preferably a solvent composed of a high boiling point organic solvent. The high boiling point organic solvent used in the invention preferably has a good compatibility with the constituent materials, especially with the monomers.

Preferable examples of the solvents include tripropylene glycol monomethyl-

ether, propylene glycol monomethylether, ethylene glycol monobutylether, diethylene glycol monobutylether, triethylene glycol monobutylether, ethylene glycol monobenzylether and diethylene glycol monobenzylether.

Although there are known low boiling point organic solvents having a boiling point of 100° C. or less, it is preferable to avoid using such solvents in consideration of unfavorable effects on the curing ability and the possibility of causing environmental pollution. In the case of using these solvents, it is preferable to select a solvent with high safety, i.e., a solvent with high control concentration (the index indicated according to the working environment evaluation standard), which is preferably 100 ppm or more and further preferably 200 ppm or more. Examples of such solvents include alcohols, ketones, esters, ethers and hydro carbons, and specifically include methanol, 2-butanol, acetone, methylethylketone, ethyl acetate, tetrahydrofuran.

The solvent can be used alone or in combination of two or more kinds. However, when water and/or a low boiling point organic solvent are used, the total amount thereof in each liquid is preferably from 0 to 20% by mass, more preferably from 0 to 10% by mass, and it is further preferable that they are substantially not contained. It is preferable that the ink and the undercoating liquid in the invention substantially does not contain water from the viewpoint of achieving temporal stability without decreasing the uniformity or increasing the turbidity of the liquid due to precipitation of a dye and the like, with the lapse of time, and from the viewpoint of securing the drying property when an impermeable or slowly permeable recording medium is used. The term "Substantially does not contain" here means that the admissible level of inevitable impurities may exist.

<Other Additives>

Known additives such as a polymer, a surface tension regulator, an ultraviolet absorber, an antioxidant, an anti-fading agent, and a pH regulator can be used in combination.

Known compounds may be appropriately selected and used as the above additives, and specific examples thereof include the additives described in JP-A 2001-181549.

Further, a pair of compounds that generate an aggregate or increase viscosity when they react with each other upon mixing can be contained separately in the ink and the undercoating liquid in the invention. The above pair of compounds has a characteristic of rapidly forming the aggregate or rapidly increasing viscosity of the liquid, thereby suppressing coalescence of adjacent liquid droplets more effectively.

Examples of the reaction of the above pair of compounds include an acid/base reaction, a hydrogen bonding reaction by a carbonic acid/amide group containing compound, a crosslinking reaction such as a reaction of boronic acid/diol, and a reaction by electrostatic interaction by cation/anion.

The following are the details of the ink jet recording device of the invention.

The ink jet recording device of the invention comprises an undercoating liquid application unit that applies an undercoating liquid containing an oligomer onto a recording medium; an undercoating liquid curing unit provided downstream of the undercoating liquid application unit and partially cures the undercoating liquid by applying energy onto at least a part of the undercoating liquid; and an image recording unit provided downstream of the undercoating liquid curing unit and records an image by ejecting, onto the partially cured undercoating liquid, an ink that is curable by irradiation of actinic energy rays.

The ink jet recording device of the invention may further comprise a conveyance unit that conveys the recording medium, and actinic energy irradiation unit provided down-

stream of the image forming unit and irradiates, with actinic energy rays, the recording medium on which an image is recorded by the image recording unit and further promotes the curing of the undercoating liquid and the ink (i.e., an image).

The image recording unit is preferably an image recording unit that ejects the ink from at least one line-formation ink jet head, the head having a length corresponding to at least the entire width of a recordable width of the recording medium and being arranged in a direction substantially perpendicular to a direction in which the recording medium is conveyed. -Mechanism of Image Recording and Recording Device-

One example of the mechanism of the invention to form an image on a recording medium while avoiding interdroplet interference will be explained by referring to FIGS. 1A to 1D.

The undercoating liquid that does not contain a coloring agent is applied onto a recording medium 16 to form a liquid film 81 of the undercoating liquid on the surface of the recording medium 16, as shown in FIG. 1A. The undercoating liquid is applied by coating in FIG. 1A, but may also be applied by ejection using an ink jet head (also referred to as "ejection"), spray coating or the like.

The thickness of the liquid film of the applied undercoating liquid is determined as an average thickness obtained by dividing the value of the volume of the applied undercoating liquid by the value of the area onto which the undercoating liquid is applied. In a case where the undercoating liquid is applied by ejection, the thickness of the liquid film can be obtained from the value of the ejected volume and the value of the area onto which the undercoating liquid has been ejected. The thickness of the liquid film of the undercoating liquid is desirably uniform with no local unevenness. From this point of view, the undercoating liquid preferably wets the recording medium well and spreads thereon, i.e., has a small degree of static surface tension, as long as the liquid can be ejected stably from the ink jet head.

After the undercoating liquid has been partially cured by irradiation with active light by a light source W (partially cured undercoating liquid (partially cured undercoating liquid layer); 81a), an ink droplet 82a is ejected as shown in FIG. 1B, thereby depositing the ink droplet 82a onto the undercoating film 81 as shown in FIG. 1C. At this time, the surface of the undercoating layer is not cured or partially cured, and has good compatibility with the ink droplet 82a.

Subsequently, another ink droplet 82b is ejected onto the recording medium 16 in the region where the layer of the undercoating liquid 81a is formed and near the position at which the first liquid droplet 82a has been ejected, as shown in FIG. 1D. At this time, the undercoating layer liquid layer 81 has a lower degree of curing at the surface thereof than in the inside thereof, thereby having good compatibility with the ink droplet 82b. Although a force works to make the ink droplet 82a and the ink droplet 82b to coalesce with each other, the interdroplet interference can be suppressed since the adhesion of the ink droplets to the surface of the undercoating layer is strong and the inside of the undercoating layer which has been cured acts as a resistance force against the coalescence between the ink droplets.

A substance that causes a chemical reaction by which a coloring material contained in the ink aggregates or becomes insoluble has conventionally been contained in the undercoating liquid, in order to avoid the interdroplet interference. However, according to the invention, the interdroplet interference can be avoided without containing such a substance in the undercoating liquid.

While the interdroplet interference is avoided and the shapes of the ink droplets of 82a and 82b are maintained (in

the case of the invention, during a period of from a few hundred milliseconds to 5 seconds) as shown in FIG. 1D, i.e., before the shapes of the droplets are lost, the ink droplets **82a** and **82b** are cured or partially cured to such a level that the shapes thereof are kept, and the color material in the ink droplets **82a** and **82b** are fixed onto the recording medium **16**. At least the ink contains an actinic energy ray curing-type polymerizable compound and is cured by a so-called polymerization reaction when irradiated with actinic energy rays such as an ultraviolet ray. The polymerization compound can also be contained in the undercoating liquid, which is preferable for promoting adhesion since the whole liquid that has been ejected is cured.

Next, the entire configuration of an inline label printer, an example of the image recording device provided with the ink jet recording device in the invention, will be explained by reference with the figures.

FIG. 2 is an entire configuration diagram showing one example of an inline label printer (image recording device) **100**. The image recording device **100** consists of an ink jet recording part **100A** in the invention, a post-processing part **100B** that performs a post-processing to the recording medium that has been recorded an image, and a buffer **104** as a cushioning unit provided between the ink jet recording part **100A** and the post-processing part **100B**.

The ink jet recording device in the invention is applied to the ink jet recording part **10A**. The ink jet recording part **100A** consists of an undercoating liquid film forming unit **100A1** that forms a partially cured undercoating liquid film that does not contain a coloring agent on the recording medium (label) **16**, and an image forming unit **100A2** that forms a desired image on the recording medium **16** by applying four inks containing a coloring material on the prescribed position of the recording medium **16**.

Favorable images can be formed particularly when a recording medium that does not have permeability (for example, OPP (Oriented Polypropylene Film), CPP (Casted Polypropylene Film), PE (Polyethylene), PET (Polyethylene Terephthalate), PP (Polypropylene), a soft wrapping material with low permeability, laminate paper, coated paper and art paper) is used as the recording medium.

In FIG. 2, the ink jet recording part **100A** is provided with the image forming unit **100A2** where an ink is applied by ink jetting onto the recording medium **16** on which the undercoating liquid has been applied with a roll coater **102P**.

The image recording device **100** is provided with a liquid storage/loading unit that is prevented from light-transmittance (not shown) and store the undercoating liquid and the ink to be supplied to the undercoating liquid film forming part **100A1** and the image forming part **100A2**; a paper supplying unit **101** that supplies the recording medium **16**; an image detecting unit **104c** that reads an image as the result of ejection of the ink (the state of the deposited ink droplets) by the image forming part **100A2**; and a rewinding unit **109** that rewinds the recorded recording medium **16**.

The paper supplying unit **101** is described in FIG. 2 as a paper supplying unit that supplies a roll paper (continuous paper), but the unit may be the type that supplies pre-cut sheets of paper.

Further details of the ink jet recording unit **100A** will now be explained. The ink jet recording unit **100A** has the image forming part **100A2** including ejecting heads **102Y**, **102C**, **102M**, and **102K** that eject ink onto the recording medium **16** in a single pass, pinning light sources **103Y**, **103C**, and **103M**, and a final curing light source **103K**; and the undercoating liquid film forming part **100A1** including the roll coater **102P** and a light source for partially curing **103P**. Specifically, it is

a so-called full-line head which is a line-formation head having a length corresponding to the entire width of the recordable area of the recording medium **16**, the head being arranged in a direction perpendicular to a direction of conveying the recording medium (shown by an arrow **S** in FIG. 2). Further, the pinning light sources **103Y**, **103C**, and **103M** are respectively arranged downstream of the ejecting heads **102Y**, **102C** and **102M**, which cure the dots of ejected ink of each color at least to such a level that the dots do not lose their shape.

The roll coater **102P** and the ejecting heads **102Y**, **102C**, **102M**, and **102K** having plural nozzles (liquid ejecting ports) are arranged in the length longer than at least one side of the recording medium **16** of the maximum size for which the ink jet recording part **100A** is intended.

The ejecting heads **102Y**, **102C**, **102M**, and **102K** corresponding to each liquid are arranged in the order of yellow ink (**Y**), cyan ink (**C**), magenta ink (**M**), and black ink (**K**) from the upstream side (the left side of FIG. 2) along with the direction **S** of conveying the recording medium, and by which a color image can be formed on the recording medium **16**.

Specifically, the undercoating liquid is first uniformly applied onto the recording medium **16** with the roll coater (**102P**), then partially curing the undercoating liquid is performed by the ultraviolet light source for partially curing **103P**. Next, the ink is ejected from the ejecting head for yellow ink **102Y** toward the recording medium **16**, then the yellow ink on the recording medium is partially cured to such a level that the surface thereof is not cured and the shape thereof is kept by the pinning light source **103Y** arranged downstream of the ejecting head **102Y**. Subsequently, the same processes as that of the yellow ink are repeated with the heads **102C** and **102M**, and after the ejection by the ejecting head for black ink **102K**, curing is completed by the final curing light source **103K** capable of completely curing the undercoating liquid and all of the inks. In this process, by partially curing the undercoating liquid and the inks after application, interdroplet interference can be avoided.

According to the image forming part **100A2** consisting of a full-line ejecting head, an image can be recorded on the entire surface of the recording medium **16** at one operation of relatively moving the recording medium **16** and the image forming part **100A2** in a direction of conveying the recording medium. Therefore, high-speed printing can be performed as compared with a case of using a shuttle type head in which the ejecting head moves back and forth in a direction perpendicular to the direction of conveying the recording medium while conveying the recording medium, thereby improving the productivity.

In the embodiments, inks of the standard colors YCMK (4 colors) are used, but the number of the colors or the combination thereof is not limited to the examples shown here, and other inks of a light color, dark color, white or other spot colors, or transparent inks may also be used depending on necessity. Examples of the possible constitutions thereof include using an ejecting head that ejects an ink of light colored type such as light cyan and light magenta in combination; delineating the background with a white ink; and adjusting the glossiness with a transparent ink.

UV light sources **103P**, **103Y**, **103C**, **103M**, and **103K** radiate ultraviolet rays to the recording medium **16** in order to cure the ink containing a polymerizable compound. Known light sources such as a medium-pressure mercury lamp, a high-pressure mercury lamp, an ultrahigh-pressure mercury lamp, a metal-halide lamp, a xenon lamp, a carbon arc lamp, an ultraviolet fluorescent lamp, an ultraviolet LED, and an ultraviolet LD can be used as the ultraviolet light source.

Among these, a high-pressure mercury lamp, an ultrahigh-pressure mercury lamp, and a metal-halide lamp are preferably used from the aspect of practicality.

The UV light source preferably has a peak of the amount of light in the wavelength range of from 200 nm to 400 nm, and preferably has an irradiation light intensity in the range of from 1 to 500 mW/cm<sup>2</sup> in the wavelength at the peak amount of light. The UV light source is preferably constituted using a cold mirror in a reflector and an infrared cut glass in a cover glass so as to prevent the increase in temperature of the recording medium by the irradiation with a heat ray. In a case of using an ink containing a radical based polymerizable compound, hindrance of the polymerization due to oxygen can be suppressed, and curing and fixing of the ink can be performed more favorably, by substituting the curing atmosphere created by the final curing light source 103K with an inert gas such as nitrogen (not shown).

An electron beam irradiation device (not shown) may also be used as a means of curing the ink containing a polymerizable compound.

In the above, the use of a UV light source and an electron beam irradiation device is discussed as a means of curing the polymerizable compound, but the means is not limited to thereto and other radiant rays such as an  $\alpha$ -x-ray,  $\gamma$ -ray, and an X-ray may also be used.

The image detecting unit 104c includes an image sensor (such as a line sensor) to pick up the image of the result of the ejection by the image forming part 100A2, and functions as a means of checking the presence of ejection abnormalities, such as clogging of the nozzles, from the image read by the image sensor.

A buffer 104 is provided as a cushioning unit between the ink jet recording part 100A and the post-processing part 100B. The recording medium that has been subjected to ink jet recording passes through the buffer 104 consisting of several upper rollers 104a and several lower rollers 104b, while repeating going up and down a few times. The buffer 104 serves as a regulator that absorbs the difference between the operation speeds (the speeds for conveying the recording medium 16) in the ink jet recording part 100A positioned upstream of the buffer and in a later-described post-processing part 100B positioned downstream of the buffer.

In the downstream of the buffer 104 is provided a varnish coater 105. In the varnish coater 105, the surface of a label is slightly coated with a varnish to improve scratch-resistance of the label surface.

A drier X is provided downstream of the varnish coater 105. For example, a UV lamp (same as the final curing light source 103K) can be used for the drier X when a UV varnish is used.

A label cutting unit 106 provided downstream of the varnish coater 105 is composed of a marking reader 106a, a die cutter driver 106b, a die cutter 106c equipped with a roll (a plate) 106e having a blade, and a facing roller 106d.

A label cut by the die cutter 106c in the label cutting unit 106 is wound up by a label winding unit 109 into the form of a product, and other parts are peeled off by a scrap removing unit 108 and disposed as a waste.

#### \*Structure of Ejecting Head

FIG. 3A is a plan perspective view showing an example of the entire basic structure of an ejecting head marked with the number 50 which is representative of the ejecting heads 102Y, 102C, 102M, and 102K.

The ejecting head 50 shown as one example in FIG. 3A is a so-called full-line head equipped with a number of nozzles 51 (liquid ejection ports) that eject a liquid toward the recording medium 16 arranged in a two-dimensional manner over a

length corresponding to the width Wm of the recording medium 16 in a direction (the main scanning direction indicated by an arrow M) which is perpendicular to a direction of conveying the recording medium 16 (the vertical scanning direction indicated by an arrow S).

In the ejecting head 50, plural pressure chamber units 54 each consisting of a nozzle 51, a pressure chamber 52 communicating to the nozzle 51 and a liquid supplying port 53 are arranged along two directions, i.e., the main scanning direction M and an inclined direction at a prescribed acute angle  $\theta$  (0 degree  $<\theta<90$  degrees) with the main scanning direction M. For illustration purpose, only a part of the pressure chamber unit 54 is shown in FIG. 3A.

The nozzles 51 are arranged at a regular pitch d in the inclined direction at a prescribed acute angle  $\theta$  with the main scanning direction M, which can be equated to that in which the nozzles are arranged in a straight line along with the main scanning direction M at an interval of "dx cos  $\theta$ ".

FIG. 3B shows a cross section along the b-b line shown in FIG. 3A of the pressure chamber unit 54 as an ejection element that constitutes the ejection head 50.

Each pressure chamber 52 communicates with a common liquid chamber 55 via the liquid supplying port 53. The common liquid chamber 55 communicates with a tank as a liquid supplying source (not shown), from which the liquid is supplied and distributed to each pressure chamber 52 via the common liquid chamber 55.

A piezoelectric body 58a is positioned on a vibrating plate 56 that forms a top face of the pressure chamber 52, and an individual electrode 57 is positioned on the piezoelectric body 58a. The vibrating plate 56 is grounded and functions as a common electrode. These vibrating plate 56, individual electrode 57 and piezoelectric body 58a constitute a piezoelectric actuator 58 that serves as a means of generating liquid ejection force.

When a prescribed driving voltage is applied to the individual electrode 57 in the piezoelectric actuator 58, the piezoelectric body 58a is deformed to change the volume of the pressure chamber 52, resulting in the change in pressure in the pressure chamber 52, and thereby a liquid is ejected from the nozzle 51. When the volume of the pressure chamber 52 returns back to the initial state after the ejection of the liquid, a new liquid is supplied to the pressure chamber 52 from the common liquid chamber 55 via the liquid supplying port 53.

In FIG. 3A, an example is shown in which a number of the nozzles 51 are arranged in a two-dimensional manner as the structure capable of forming an image with high resolution on the recording medium 16 at high speed. However, the structure of the ejecting head in the invention is not particularly limited to the above structure and may be a structure in which the nozzles are arranged in a one-dimensional manner. The structure of the pressure chamber unit 54 as an ejection element that constitutes the ejecting head is also not particularly limited to the example shown in FIG. 3B. For example, the common liquid chamber 55 may be positioned above the pressure chamber 52 (i.e., the opposite side of the ejection face 50a) instead of positioning the same under the pressure chamber 52 (i.e., the ejection face 50a side of the pressure chamber 52). Further, the liquid ejection force may be generated by an exothermic body instead of the piezoelectric body 58a.

In the ink jet recording device in the invention, other devices such as ejection of the undercoating liquid from the nozzle may also be used for the application of the undercoating liquid onto the recording medium, instead of coating.

The device used for the coating is not particularly limited, and known coating devices can be selected as appropriate

according to usage. Examples thereof include an air doctor coater, a blade coater, a rod coater, a knife coater, a squeeze coater, an impregnating coater, a reverse roll coater, a transfer roll coater, a gravure coater, a kiss roll coater, a cast coater, a spray coater, a curtain coater, and an extruding coater.

\*Liquid Supply System

FIG. 4 is a schematic view showing a configuration of the liquid supply system in the image recording device 100.

A liquid tank 60 supplies a liquid to the ejecting head 50 as a base tank. In the midstream of a tube that connects the liquid tank 60 and the ejecting head 50, a liquid supplying pump 62 that sends the liquid to the ejecting head 50 is provided. The tube, liquid tank 60 and the ejecting head 50 preferably have a temperature which is regulated together with the ink contained therein, by a temperature detecting means and a heater. The ink temperature is preferably regulated to a range of from 40° C. to 80° C.

The image recording device 100 is provided with a cap 64 as a means for preventing a meniscus of the nozzle 51 from drying during the intermission of ejection, or from increasing in viscosity in the vicinity of the meniscus, and a cleaning blade 66 as a means for cleaning the ejection face 50a. A maintenance unit including the cap 64 and the cleaning blade 66 can be transferred relatively to the ejecting head 50 by a transfer system (not shown), and can be transferred to a maintenance position positioned below the ejecting head 50 from a prescribed retracting position as necessary.

The cap 64 is elevated relatively to the ejecting head 50 with an elevation mechanism (not shown). The elevation mechanism is designed to cover at least the region of the nozzle in the ejection face 50a with the cap 64, by elevating the cap 64 up to a prescribed position and attaching the cap 64 to the ejecting head 50.

The cap 64 preferably has the inside thereof divided into plural areas each corresponding to each row of the nozzles by dividing walls, and each of the divided areas can be selectively suctioned using a selector or the like.

The cleaning blade 66 is composed of an elastic member such as rubber, and is capable of sliding on the ejection face 50a of the ejecting head 50 with a transfer mechanism for the cleaning blade (not shown). When the liquid droplets or foreign materials are attached onto the ejection face 50a, the ejection face 50a is wiped off by sliding the cleaning blade 66 on the ejection face 50a and cleaned.

A suction pump 67 sucks a liquid from the nozzle 51 of the ejecting head 50 while the ejection face 50a of the ejecting head 50 is covered with the cap 64, and sends the sucked liquid to a collection tank 68.

The above suction operation is also performed when the liquid tank 60 is loaded in the image recording device 100 and the liquid tank 60 is filled with a liquid from the liquid tank 60 (at the time of the initial filling) or when the liquid having viscosity that has been increased during the long-term cessation is removed (at the time of starting the operation after a long-term intermission).

Note that there are two types of ejections from the nozzle: first, a normal ejection performed onto a recording medium such as paper in order to form an image; and second, a purge performed onto the cap 64 serving as a liquid receiver (also referred to as a blank ejection).

Further, when air bubbles are mixed into the nozzle 51 or the pressure chamber 52 in the ejecting head 50 or increase in the viscosity in the nozzle 51 exceeds a certain level, the liquid cannot be ejected from the nozzle 51 by the above-described blank ejection. In this case, the liquid with the air bubbles or increased viscosity in the pressure chamber 52 in

the ejecting head 50 is sucked by the suction pump 67 by applying the cap 64 onto the ejection face 50a in the ejecting head 50.

The ejecting head 50, liquid tank 60, liquid supplying pump 62, cap 64, cleaning blade 66, suction pump 67, collection tank 68 and an ink flowing route that connects these units, as well as other members and equipments with which the ink directly contact, preferably have dissolution resistance and swelling resistance. Further, these members and equipments preferably have a light shielding property.

\*Control System

FIG. 5 is a block diagram of the main part showing a system configuration of the image recording device 100.

In FIG. 5, the image recording device 100 is mainly composed of an image forming unit 102, image detecting unit 104c, UV light source 103, communication interface 110, system controller 112, memory 114, image buffer memory 152, motor for transportation 116, motor driver 118, heater 122, heater driver 124, medium type detecting unit 132, ink type detecting unit 134, illumination intensity detecting unit 135, environmental temperature detecting unit 136, environmental humidity detecting unit 137, medium temperature detecting unit 138, liquid supplying unit 142, liquid supplying driver 144, printing control unit 150, head driver 154, and a light source driver 156.

Since the image forming unit 102 is shown as a representative of the ejecting heads 102Y, 102C, 102M and 102K shown in FIG. 2, the UV light source is shown as a representative of the curing light sources 103P, 103Y, 103C, 103M and 103K shown in FIG. 2, and the image detecting unit 104c is the same as the one described in FIG. 2 which have been mentioned above, further explanation thereof is omitted here.

The communication interface 110 is an image data inputting means that receives the image data sent from a host computer 300. For the communication interface 110, wired interfaces such as USB (Universal Serial Bus) or IEEE1394, or wireless interfaces can be applied. The image data inputted into the image recording device 100 via the communication interface 110 are temporarily memorized in a first memory 114 for memorizing image data.

The system controller 112 is composed of a central processing unit (CPU), its surrounding circuit, and the like, and is a main controlling means of controlling the entire image recording device 100 according to a prescribed program that has been previously memorized in the first memory 114. That is, the system controller 112 controls each unit of the communication interface 110, motor driver 118, heater driver 124, medium type detecting unit 132, ink type detecting unit 134, printing control unit 150 and the like.

The motor for transportation 116 imparts a driving force to rollers, belts or the like that transport a recording medium. By this motor for transportation 116, the ejecting head 50 that constitutes the image forming unit 102 and the recording medium move relatively to each other. The motor driver 118 is a circuit that drives the motor for transportation 116 in accordance with the instructions given from the system controller 112.

The heater 122 is a circuit that drives a heater (or a cooling element) 122 which is not shown in the Figure, and maintains the temperature of the recording medium to be constant. The heater driver 124 is a circuit that drives the heater 122 in accordance with the instructions given from the system controller 112.

The medium type detecting unit 132 detects the type of the recording medium. There are various embodiments of detecting the type of the recording medium, and examples thereof include an embodiment of detecting the type by a sensor

provided at a paper supplying unit which is not shown in the Figure; an embodiment of inputting the type by the operation of a user; an embodiment of inputting the type from the host computer 300; and an embodiment in which the type is automatically detected by analyzing the image data (for example, resolution or color) inputted from the host computer 300 or supplemental data of the image data.

The ink type detecting unit 134 detects the type of the ink. There are various embodiments of detecting the type of the ink and examples thereof include an embodiment of detecting by a sensor provided in the liquid storage/loading unit which is not shown in the Figure; an embodiment of inputting the type by the operation of a user; an embodiment of inputting the type from the host computer 300; and an embodiment in which the type is automatically detected by analyzing the image data (for example, resolution or color) inputted from the host computer 300 or supplemental data of the image data.

The illumination intensity detecting unit 135 detects the illumination intensity of the UV rays emitted from the UV light source 103. Examples of the embodiments of detecting the illumination intensity include an embodiment of detecting the illumination intensity by a sensor provided near the UV light source 103 shown in FIG. 2. The feedback of the output of this illumination intensity sensor is sent to the output of the UV light source.

The environmental temperature detecting unit 136 detects the temperatures of the outside air and the inside of the image recording device. Examples of the embodiments of detecting the environmental temperature include an embodiment of detecting the environmental temperature by a sensor provided at the outside or inside of the device.

The environmental humidity detecting unit 137 detects the humidity of the outside air and the inside of the image recording device. Examples of the embodiments of detecting the environmental humidity include an embodiment of detecting the humidity by a sensor provided at the outside or the inside of the device.

The medium temperature detecting unit 138 detects the temperature of the recording medium at the time of forming an image. There are various embodiments of detecting the medium temperature and examples thereof include an embodiment of detecting the temperature by a contact type temperature sensor and an embodiment of detecting the temperature by a non-contact type temperature sensor provided above the recording medium 16. The temperature of the recording medium is maintained constant by the heater 122.

The liquid supplying unit 142 is composed of a tube through which the ink flows from the liquid tank 60 shown in FIG. 4 to the image forming unit 102, the liquid supplying pump 62, and the like.

The liquid supplying driver 144 is a circuit that drives the liquid supplying pump that constitutes the liquid supplying unit and the like so that the liquid can be supplied to the image forming unit 102.

The printing control unit 150 produces the data (ejection data) necessary for each ejecting head 50 that constitute the image forming unit 102 to perform ejection (jetting) toward the recording medium based on the image data inputted in the image recording device 100. That is, the printing control unit 150 functions as an image processing means that performs image processing such as various processes, corrections or the like to generate the ejection data from the image data stored in the first memory 114 in accordance with the control of the system controller 112, and supplies the generated ejection data to the head driver 154.

The printing control unit 150 is accompanied with a second memory 152, and the ejection data and the like are tempo-

rarily stored in the second memory 152 at the time of performing the image processing in the printing control unit 150.

In FIG. 5, the second memory 152 is shown as an embodiment in which it accompanies the printing control unit 150. However, the first memory 114 can also function as the second memory 152 at the same time. Further, the printing control unit 150 and the system controller 112 can also be integrated and configured with a single processor.

The head driver 154 outputs a driving signal for the ejection to each ejecting head 50 that constitute the image forming unit 12 based on the ejection data given from the printing control unit 150 (practically, it is the ejection data stored in the second memory 152). The driving signal for the ejection outputted from this head driver 154 is given to each ejecting head 50 (specifically, the actuator 58 shown in FIG. 3B), the liquid (liquid droplets) is ejected onto the recording medium from the ejecting head 50.

A light source driver 156 is a circuit that controls the voltage, time and the timing to be inputted in the UV light source 103 based on the instructions given from the printing control unit 150, illumination intensity detected by the illumination intensity detecting unit 135, environmental temperature detected by the environmental temperature detecting unit 136, environmental humidity detected by the environmental humidity detecting unit 137 and the medium temperature detected by the medium temperature detecting unit 138, and drives the UV light source 103.

The following are the exemplary embodiments according to the invention:

1. An ink jet recording method comprising:  
applying an undercoating liquid comprising an oligomer onto a recording medium;  
partially curing the undercoating liquid that has been applied onto the recording medium; and  
recording an image by ejecting onto the partially cured undercoating liquid an ink that is curable by irradiation with actinic energy rays.
2. The ink jet recording method of 1, wherein the oligomer is a urethane acrylate oligomer.
3. The ink jet recording method of 1, wherein the undercoating liquid is cured by irradiation with actinic energy rays.
4. The ink jet recording method of 1, wherein the undercoating liquid further comprises a radical polymerizable composition.
5. The ink jet recording method of 1, wherein the image is recorded with a multi-color ink set, and the method further comprises partially curing the ink of at least one color ejected onto the recording medium.
6. The ink jet recording method of 1, further comprising promoting the curing of the ink and the undercoating liquid.
7. The ink jet recording method of 1, wherein the curing sensitivity of the ink is equal to or higher than the curing sensitivity of the undercoating liquid.
8. The ink jet recording method of 1, wherein the internal viscosity at 25° C. of the partially cured undercoating liquid is at least 1.5 times the viscosity at 25° C. at the surface of the partially cured undercoating liquid.
9. The ink jet recording method of 1, wherein the recording medium is non-permeable or slowly permeable.
10. The ink jet recording method of 1, wherein the undercoating liquid is applied by a coater.
11. An ink jet recording device comprising:  
an undercoating liquid application unit that applies an undercoating liquid containing an oligomer onto a recording medium;

an undercoating liquid curing unit that is provided downstream of the undercoating liquid application unit and that partially cures the undercoating liquid by applying energy thereto; and

an image recording unit that is provided downstream of the undercoating liquid curing unit and that forms an image by ejecting, onto the partially cured undercoating liquid, an ink that is curable by irradiation with actinic energy rays.

12. The ink jet recording device of 11, further comprising: a conveyance unit that conveys the recording medium; and

an actinic energy rays irradiation unit that is provided downstream of the image recording unit in the direction in which the recording medium is conveyed, and that irradiates, with actinic energy rays, the recording medium on which an image has been recorded by the image recording unit and further promotes the curing of the ink and the undercoating liquid, wherein:

the image recording unit ejects the ink from at least one full-line ink jet head, the head having a length corresponding to at least the entire width of a recordable width of the recording medium and the head being arranged in a direction substantially perpendicular to the direction in which the recording medium is conveyed.

13. The ink jet recording device of 11, wherein the oligomer is a urethane acrylate oligomer.

14. The ink jet recording device of 11, wherein the undercoating liquid is cured by irradiation with actinic energy rays.

15. The ink jet recording device of 11, wherein the undercoating liquid further comprises a radical polymerizable composition.

16. The ink jet recording device of 11, wherein the image is recorded with a multi-color ink set, and the ink jet recording device carries out partially curing of the ink of at least one color that has been ejected onto the recording medium.

17. The ink jet recording device of 11, wherein the curing sensitivity of the ink is equal to or higher than the curing sensitivity of the undercoating liquid.

18. The ink jet recording device of 11, wherein the internal viscosity at 25° C. of the partially cured undercoating liquid is at least 1.5 times the viscosity at 25° C. at the surface of the partially cured undercoating liquid.

19. The ink jet recording device of 11, wherein the recording medium is non-permeable or slowly permeable.

20. The ink jet recording device of 11, wherein the undercoating liquid is applied by a coater.

## EXAMPLES

Further details of the invention will now be explained by Examples. However, the invention is not limited to the following examples as long as its main purport is not exceeded.

### Example 1

#### <Preparation of Cyan Pigment Dispersion P-1>

PB15:3 (trade name: IRGALITE BLUE GLO, a pigment manufactured by Ciba Specialty Chemicals K.K.) 16 g, dipropylene glycol diacrylate (DPGDA, manufactured by DAICEL-CYTEC Company, Ltd) 48 g, and SOLSPERSE 32000 (a dispersant manufactured by Zeneca) 16 g were mixed with a stirrer for an hour. The resulting mixture was then dispersed with an Eiger mill and a cyan pigment dispersion P-1 was obtained.

The dispersion was conducted under the conditions that the mill was filled with zirconia beads having a diameter of 0.65 mm at a filling rate of 70%, the peripheral velocity was 9 m/s, and the dispersion time was 1 hours.

#### <Preparation of Cyan Ink Jet Recording Liquid I-1>

The following components were mixed by stirring and dissolved, and a cyan ink jet recording liquid I-1 was prepared. The surface tension at 25° C. of the cyan ink jet recording liquid I-1 was 27 mN/m, and the viscosity at 25° C. thereof was 15 mPa·s.

##### -Components-

Pigment dispersion P-1 2.16 g

Dipropylene glycol diacrylate (polymerizable compound, DPGDA; manufactured by DAICEL-CYTEC Company, Ltd) 9.84 g

Irg 907 (a photopolymerization initiator shown below; manufactured by Ciba Specialty Chemicals K.K.) 1.5 g

DAROCURE ITX (a sensitizer shown below; manufactured by Ciba Specialty Chemicals K.K.) 0.75 g

DAROCURE EDB (a sensitizer shown below; manufactured by Ciba Specialty Chemicals K.K.) 0.75 g



#### <Preparation of Magenta Pigment Dispersion P-2>

The magenta pigment dispersion P-2 was prepared in the same manner as the preparation of the cyan pigment dispersion P-1, except that a pigment PV 19 (CINQUASIA MAZENTA RT-355D; manufactured by Ciba Specialty Chemicals K.K.) and a dispersant DISPERBYK 168 (manufactured by BYK-Chemie Japan K.K.) were used instead of PB15:3 and SOLSPERSE 32000, respectively.

#### <Preparation of Yellow Pigment Dispersion P-3>

The yellow pigment dispersion P-3 was prepared in the same manner as the preparation of the cyan pigment dispersion P-1, except that a pigment PY 120 (NOVOPERM YELLOW H2G; manufactured by Clariant Japan K.K.) and a dispersant DISPERBYK 168 (manufactured by BYK-Chemie Japan K.K.) were used instead of PB 15:3 and SOLSPERSE 32000, respectively.

#### <Preparation of Black Pigment Dispersion P-4>

The black pigment dispersion P-4 was prepared in the same manner as the preparation of the cyan pigment dispersion P-1, except that a carbon black (SPECIAL BLACK 250; manufactured by Degussa Japan Co., Ltd.) and a dispersant SOLSPERSE 5000 (manufactured by Zeneca) were used instead of PB 15:3 and SOLSPERSE 32000, respectively.

#### <Preparation of Magenta Ink Jet Recording Liquid I-2>

The following components were mixed by stirring and dissolved, and a magenta ink jet recording liquid I-2 was prepared. The surface tension at 25° C. of the magenta ink jet recording liquid I-2 was 27 mN/m, and the viscosity at 25° C. thereof was 16 mPa·s.

## -Components-

Pigment dispersion P-2 5.86 g

Dipropylene glycol diacrylate (a polymerizable compound, DPGDA; manufactured by DAICEL-CYTEC Company, Ltd) 6.14 g

Irg 907 (a photopolymerization initiator shown below; manufactured by Ciba Specialty Chemicals K.K.) 1.5 g

DAROCURE ITX (a sensitizer shown below; manufactured by Ciba Specialty Chemicals K.K.) 0.75 g

DAROCURE EDB (a sensitizer shown below; manufactured by Ciba Specialty Chemicals K.K.) 0.75 g

## &lt;Preparation of Yellow Ink Jet Recording Liquid I-3&gt;

The following components were mixed by stirring and dissolved, and a yellow ink jet recording liquid I-3 was prepared. The surface tension at 25° C. of the yellow ink jet recording liquid I-3 was 27 mN/m, and the viscosity at 25° C. thereof was 16 mPa·s.

## -Components-

Pigment dispersion P-3 4.68 g

Dipropylene glycol diacrylate (polymerizable compound, DPGDA; manufactured by DAICEL-CYTEC Company, Ltd) 7.32 g

Irg 907 (a photopolymerization initiator shown below; manufactured by Ciba Specialty Chemicals K.K.) 1.5 g

DAROCURE ITX (a sensitizer shown below; manufactured by Ciba Specialty Chemicals K.K.) 0.75 g

DAROCURE EDB (a sensitizer shown below; manufactured by Ciba Specialty Chemicals K.K.) 0.75 g

## &lt;Preparation of Black Ink Jet Recording Liquid I-4&gt;

The following components were mixed by stirring and dissolved, and a black ink jet recording liquid I-4 was prepared. The surface tension at 25° C. of the black ink jet recording liquid I-4 was 27 mN/m, and the viscosity at 25° C. thereof was 15 mPa·s.

## -Components-

Pigment dispersion P-4 3.3 g

Dipropylene glycol diacrylate (polymerizable compound, DPGDA; manufactured by DAICEL-CYTEC Company, Ltd) 8.7 g

Irg 907 (a photopolymerization initiator shown below; manufactured by Ciba Specialty Chemicals K.K.) 1.5 g

DAROCURE ITX (a sensitizer shown below; manufactured by Ciba Specialty Chemicals K.K.) 0.75 g

DAROCURE EDB (a sensitizer shown below; manufactured by Ciba Specialty Chemicals K.K.) 0.75 g

## &lt;Preparation of Undercoating Liquid II-1&gt;

The following components were mixed by stirring and dissolved, and the undercoating liquid II-1 that does not contain an oligomer. The surface tension at 25° C. of the undercoating liquid II-2 was 22 mN/m, and the viscosity at 25° C. thereof was 12 mPa·s.

## -Components-

Dipropylene glycol diacrylate (polymerizable compound, DPGDA; manufactured by DAICEL-CYTEC Company, Ltd) 11.85 g

Irg 907 (a photopolymerization initiator shown below; manufactured by Ciba Specialty Chemicals K.K.) 1.5 g

DAROCURE ITX (a sensitizer shown below; manufactured by Ciba Specialty Chemicals K.K.) 0.75 g

DAROCURE EDB (a sensitizer shown below; manufactured by Ciba Specialty Chemicals K.K.) 0.75 g

BYK-307 (manufactured by BYK-Chemie Japan K.K.) 0.15 g

## &lt;Preparation of Undercoating Liquids II-2 to II-14&gt;

The undercoating liquids II-2 to II-14 were prepared in the same manner with the preparation of the undercoating liquid

II-1, except that the oligomers (the kind and addition amount thereof are shown in the following Table 1) were further added, respectively.

In the above preparation process, the addition amount of the DPGDA was reduced in accordance with the addition amount of the oligomer to be added so that the total amount of the undercoating liquid was 15 g.

TABLE 1

| Undercoating Liquid Standard | Type                                | Oligomer |                                                                   |
|------------------------------|-------------------------------------|----------|-------------------------------------------------------------------|
|                              |                                     |          | Addition amount [mass %: with respect to the undercoating liquid] |
| II-1                         | —                                   | —        | —                                                                 |
| II-2                         | R1204 (urethane acrylate)           | 30%      | 30%                                                               |
| II-3                         | R1901 (urethane acrylate)           | 30%      | 30%                                                               |
| II-4                         | Ebecryl 230 (urethane acrylate)     | 30%      | 30%                                                               |
| II-5                         | Ebecryl 270 (urethane acrylate)     | 30%      | 30%                                                               |
| II-6                         | Ebecryl 4858 (urethane acrylate)    | 30%      | 30%                                                               |
| II-7                         | Ebecryl 8210 (urethane acrylate)    | 30%      | 30%                                                               |
| II-8                         | Ebecryl 210 (urethane acrylate)     | 30%      | 30%                                                               |
| II-9                         | Ebecryl 4827 (urethane acrylate)    | 30%      | 30%                                                               |
| II-10                        | Ebecryl 6700 (urethane acrylate)    | 30%      | 30%                                                               |
| II-11                        | Ebecryl 4450 (urethane acrylate)    | 30%      | 30%                                                               |
| II-12                        | Ebecryl IRR467 (polyester acrylate) | 30%      | 30%                                                               |
| II-13                        | Ebecryl 810 (polyester acrylate)    | 30%      | 30%                                                               |
| II-14                        | Ebecryl IRR302 (polyester acrylate) | 30%      | 30%                                                               |

## 30 Notes:

R1204 and R1901 are the products of DAI-ICHI KOGYO SEIYAKU CO., LTD.

Ebecryl Series are the products of DAICEL-CYTEC Company LTD.

The surface tensions and viscosities of the above undercoating liquids II-2 to II-14 are shown in the following Table 2.

TABLE 2

| Undercoating Liquid Standard | Surface Tension [mN/m] | Viscosity [mPa·s] |
|------------------------------|------------------------|-------------------|
| II-2                         | 22                     | 120               |
| II-3                         | 22                     | 92                |
| II-4                         | 22                     | 52                |
| II-5                         | 22                     | 93                |
| II-6                         | 22                     | 39                |
| II-7                         | 22                     | 27                |
| II-8                         | 22                     | 91                |
| II-9                         | 22                     | 92                |
| II-10                        | 22                     | 130               |
| II-11                        | 22                     | 41                |
| II-12                        | 22                     | 110               |
| II-13                        | 22                     | 24                |
| II-14                        | 22                     | 95                |

55 In the Examples, the surface tensions were measured by a surface tensiometer (CBVP-Z, manufactured by KYOWA INTERFACE SCIENCE CO., LTD.), and the viscosity was measured by a portable digital viscometer for laboratory use (VISCOSTICK, manufactured by MARUYASU INDUSTRIES Co., Ltd.)

## &lt;Image Recording and Evaluation&gt;

60 An experimental apparatus having the following units was prepared for an image recording apparatus: a conveying unit that conveys a recording medium by rotating a driving roll; a roll coater that applied an undercoating liquid on the recording medium; a light source that partially cures the applied undercoating liquid consisting of an array of extra-high voltage mercury lamps arranged in parallel with a direction perpendicular to a direction in which the recording medium is

conveyed, i.e., the main scanning direction (in a width direction) upon recording onto the recording medium; an ink jet printing device that records an image mounted with four full-line head sets, wherein each head set consists of a head (manufactured by TOSHIBA TEC CORPORATION, droplet frequency; 6.2 KHz, number of nozzles; 636, nozzle density; 300 dpi (nozzle/inch, hereinafter the same), droplet size; from 6 pL to 42 pL which is changeable in seven levels); and a metal halide lamp that irradiates with actinic energy rays to perform further curing of the undercoating liquid and the recorded image.

On a conveyor route for the recording medium, the roll coater and the light source that partially cures the undercoating liquid are arranged in this order from upstream to downstream, as shown in FIG. 2, and the head unit having four heads for yellow, cyan, magenta and black and the extra-high mercury lamps that half-cure the ink are arranged downstream of the light source, wherein each of the light sources is respectively arranged downstream of each head, in such a manner that the recording medium can be conveyed right under the heads. The heads are fixed to the apparatus in the order of yellow, cyan, magenta and black, from upstream of the direction in which a recording medium is conveyed. Further, the metal halide lamp is provided downstream of the head for black.

In this Example, the experimental apparatus was charged with the undercoating liquid II-1 and the ink jet recording liquids I-1 to I-4 of four colors in the ink jet printing part thereof, then an image of 300 dpi×600 dpi was recorded onto the recording medium in accordance with the method as described below.

First, the undercoating liquid was uniformly applied to a thickness of 5  $\mu\text{m}$  by a roll coater (application rate; 400 mm/s). After the application of the undercoating liquid, exposure was performed with the light source for partially curing the undercoating liquid (light intensity; 500 mW/cm<sup>2</sup>), then the applied undercoating liquid was partially cured.

At this time, the portion ranging from the surface to a point 1  $\mu\text{m}$  from the surface in depth of the undercoating liquid on the recording medium was partially cured, and the internal side thereof was completely cured. The partially cured surface portion was scraped together and the viscosity at 25°C. thereof was measured by a portable digital viscometer for laboratory use (VISCOSTICK, manufactured by MARUYASU INDUSTRIES Co., Ltd.). The viscosity of the surface portion was 1000 mPa·s.

A transferring test was conducted using a plain paper sheet as a permeable medium (copy paper C2, product code; V436, manufactured by FUJI XEROX CO., LTD.). The paper sheet was pressed against a partially cured undercoating liquid or colored liquid on a sample recording medium with uniform force (500 mN/cm<sup>2</sup>) and left for about a minute. Thereafter, the paper sheet was gently peeled off and measured the weight thereof to calculate the amount of uncured liquid.

When an image was formed with a droplet size of 24 pL, the amount of the uncured liquid was in the range of from 0.20 mg/cm<sup>2</sup> to 0.24 mg/cm<sup>2</sup>. In the invention, the maximum mass per area of the ejected ink "m" was from 1.48 mg/cm<sup>2</sup> to 1.74 mg/cm<sup>2</sup>, when an image of 600 dpi×600 dpi was formed with a droplet size of 24 pL.

Accordingly, the mass per area of the uncured undercoating liquid "M (undercoating liquid)" and the maximum mass per area of the ejected recording liquid "m (recording liquid)" satisfied the relation "m (recording liquid)/10<M (undercoating liquid)<m (recording liquid)/5".

Subsequently, the ink jet recording liquids I-1 to I-4 were respectively ejected onto the recording medium on which the

undercoating liquid has been applied, by the heads charged with the ink jet recording liquids I-1 to I-4 (here, irradiation for partially curing the ink by the extra-high voltage mercury lamps provided together was not performed), and the liquids 5 were cured by irradiating an ultraviolet ray having a wavelength of 365 nm at a light intensity of 3000 mW/cm<sup>2</sup> with the metal halide lamp.

In this way, mono-color images were printed in the form of dots of 150 dpi in the main scanning direction and 150 dpi in 10 the sub scanning direction (one drop is used, droplet size; 6 pL), and in the form of a solid image of 600 dpi in a main scanning direction and 300 dpi in a sub-scanning direction (four drops are used, droplet size; 24 pL), by ejecting each of the ink jet recording liquids I-1 to I-4, separately.

15 Further, after application and partially curing the undercoating layer in the same manner as described above, a full-color image of a woman of 300 dpi in a main scanning direction and 600 dpi in a sub-scanning direction was printed onto the recording medium using all of the ink jet recording liquid I-1 to I-4 by a head charged with the ink jet recording liquids I-1 to I-4 (conveying rate of the recording medium; 400 mm/s, printed with four tones of from 6 to 24 pL, an anti-aliasing process was performed). In this process, pinning exposure was repeated after each ejection of each color by the 20 extra-high voltage mercury lamps (light intensity; 500 mW/cm<sup>2</sup>), and the inks of each color was partially cured. Thereafter, an ultraviolet ray (wavelength; 365 nm) was irradiated at a light intensity of 3000 mW/cm<sup>2</sup> by the metal halide lamp, thereby fixing the image.

25 The maximum mass per area of the ejected ink "m" was in the range of 1.48 mg/cm<sup>2</sup> to 1.74 mg/cm<sup>2</sup> when an image of 600 dpi×600 dpi was formed with a droplet size of 24 pL.

30 Further, the amount of the uncured yellow liquid after pinning exposure, the amount of the uncured cyan liquid after 35 pinning exposure, and the amount of the uncured magenta liquid after pinning exposure were measured by sampling after each process and conducting transferring test. In each case of the above liquids, the amount of the uncured liquid was in the range of from 0.20 mg/cm<sup>2</sup> to 0.24 mg/cm<sup>2</sup>, when 40 an image was formed with a droplet size of 24 pL.

Accordingly, in the case of a combination of liquids having different colors, the mass per area of the uncured undercoating liquid A, which is ejected onto the recording medium first, "M (liquid A)" and the maximum mass per area of the ejected 45 recording liquid B, which is ejected onto the recording medium after the liquid A, "m (liquid B)" satisfied the relation "m (liquid B)/10<M (liquid A)<m (liquid B)/5".

In the above process, the interval between the completion 50 of application of the undercoating liquid and the ejection of the first color liquid (the yellow ink jet recording liquid I-3) was set at 0.2 second. LINTEC YUPO 80 (manufactured by Lintec Corporation) and OJITAC NYUPO (manufactured by OJITAC Co., Ltd.) were used as the recording media.

55 After the recording of the image using the undercoating liquid II-1, the same processes were performed by using the above-mentioned undercoating liquids II-2 to II-14 instead of the undercoating liquid II-1.

The obtained mono-color images were sliced and observed by an optical microscope (measuring microscope MM-40, 60 manufactured by Nikon Corporation). The slices was obtained using a microtome (RM2255; manufactured by Leica Microsystems Japan).

In an image portion of the obtained image, as shown in FIG. 6, the cured portion of the recording liquid 24 was partly 65 exposed on the surface 22 and partly submerged in the undercoating liquid layer 20, and the undercoating liquid layer 20 existed under the cured portion of the recording liquid 24.

Further, it was observed that a uniform layer of the cured portion of the recording liquid **24** was formed.

In the same manner, in a portion of the full color image as shown in FIG. 8, the cured portion of the recording liquid **28** was partly exposed on the surface **22** and partly submerged in the layer of the other recording liquid **24**, and the layer of the other recording liquid **24** existed under the undercoating liquid layer **28**. Further, it was observed that a uniform layer of the cured portion of the recording liquid **28** was formed.

Measurement and evaluation of the obtained images were performed. The results are shown in Tables 3 to 7.

### 1. Evaluation of Solid Images

The solid images were evaluated by visual observation in accordance with the following criteria:

A: No white spots were observed over the whole image.

B: White spots (5 Mm or smaller) were slightly observed.

C: White spots (greater than 5  $\mu$ m) were distinctively observed.

### 2. Evaluation of Dot Diameters

The dot diameters of the dot pattern images of 150 dpi $\times$ 150 dpi were measured using a dot analyser DA 6000 (manufactured by Oji Scientific Instruments).

### 3. Evaluation of Practical Images

The full-color images of a woman were evaluated by visual observation in accordance with the following criteria:

A: A favorable image with sufficient density and sharpness was obtained.

B: Regions with high density (e.g., the hair of the woman) appeared pale in some degree.

C: The color tone over the whole image appeared pale.

D: The image appeared indistinct.

E: Unevenness was observed in the image.

TABLE 3

| Undercoating Liquid | YUPO 80      |             | N YUPO       |             | Notes         |
|---------------------|--------------|-------------|--------------|-------------|---------------|
|                     | Dot diameter | Solid image | Dot diameter | Solid image |               |
| II-1                | 50 $\mu$ m   | C           | 50 $\mu$ m   | C           | Comp. Example |
| II-2                | 60 $\mu$ m   | A           | 60 $\mu$ m   | A           | the Invention |
| II-3                | 60 $\mu$ m   | A           | 60 $\mu$ m   | A           | the Invention |
| II-4                | 60 $\mu$ m   | A           | 60 $\mu$ m   | A           | the Invention |
| II-5                | 60 $\mu$ m   | A           | 60 $\mu$ m   | A           | the Invention |
| II-6                | 60 $\mu$ m   | A           | 60 $\mu$ m   | A           | the Invention |
| II-7                | 60 $\mu$ m   | A           | 60 $\mu$ m   | A           | the Invention |
| II-8                | 60 $\mu$ m   | A           | 60 $\mu$ m   | A           | the Invention |
| II-9                | 60 $\mu$ m   | A           | 60 $\mu$ m   | A           | the Invention |
| II-10               | 60 $\mu$ m   | A           | 60 $\mu$ m   | A           | the Invention |
| II-11               | 60 $\mu$ m   | A           | 60 $\mu$ m   | A           | the Invention |
| II-12               | 55 $\mu$ m   | B           | 55 $\mu$ m   | B           | the Invention |
| II-13               | 55 $\mu$ m   | B           | 55 $\mu$ m   | B           | the Invention |
| II-14               | 55 $\mu$ m   | B           | 55 $\mu$ m   | B           | the Invention |
| None                | 45 $\mu$ m   | C           | 80 $\mu$ m   | A           | Comp. Example |

TABLE 4

| Undercoating Liquid | YUPO 80      |             | N YUPO       |             | Notes         |
|---------------------|--------------|-------------|--------------|-------------|---------------|
|                     | Dot diameter | Solid image | Dot diameter | Solid image |               |
| II-1                | 50 $\mu$ m   | C           | 50 $\mu$ m   | C           | Comp. Example |

TABLE 4-continued

| 5  | <Magenta Ink>       |              |             |              |             |               |
|----|---------------------|--------------|-------------|--------------|-------------|---------------|
|    | Undercoating Liquid | YUPO 80      |             | N YUPO       |             | Notes         |
|    |                     | Dot diameter | Solid image | Dot diameter | Solid image |               |
| 10 | II-2                | 60 $\mu$ m   | A           | 60 $\mu$ m   | A           | the Invention |
| 15 | II-3                | 60 $\mu$ m   | A           | 60 $\mu$ m   | A           | the Invention |
| 15 | II-4                | 60 $\mu$ m   | A           | 60 $\mu$ m   | A           | the Invention |
| 15 | II-5                | 60 $\mu$ m   | A           | 60 $\mu$ m   | A           | the Invention |
| 15 | II-6                | 60 $\mu$ m   | A           | 60 $\mu$ m   | A           | the Invention |
| 15 | II-7                | 60 $\mu$ m   | A           | 60 $\mu$ m   | A           | the Invention |
| 15 | II-8                | 60 $\mu$ m   | A           | 60 $\mu$ m   | A           | the Invention |
| 15 | II-9                | 60 $\mu$ m   | A           | 60 $\mu$ m   | A           | the Invention |
| 15 | II-10               | 60 $\mu$ m   | A           | 60 $\mu$ m   | A           | the Invention |
| 15 | II-11               | 60 $\mu$ m   | A           | 60 $\mu$ m   | A           | the Invention |
| 15 | II-12               | 55 $\mu$ m   | B           | 55 $\mu$ m   | B           | the Invention |
| 15 | II-13               | 55 $\mu$ m   | B           | 55 $\mu$ m   | B           | the Invention |
| 15 | II-14               | 55 $\mu$ m   | B           | 55 $\mu$ m   | B           | the Invention |
| 20 | None                | 45 $\mu$ m   | C           | 80 $\mu$ m   | A           | Comp. Example |

TABLE 5

| 25 | <Yellow Ink>        |              |             |              |             |               |
|----|---------------------|--------------|-------------|--------------|-------------|---------------|
|    | Undercoating Liquid | YUPO 80      |             | N YUPO       |             | Notes         |
|    |                     | Dot diameter | Solid image | Dot diameter | Solid image |               |
| 30 | II-1                | 50 $\mu$ m   | C           | 50 $\mu$ m   | C           | Comp. Example |
| 30 | II-2                | 60 $\mu$ m   | A           | 60 $\mu$ m   | A           | the Invention |
| 30 | II-3                | 60 $\mu$ m   | A           | 60 $\mu$ m   | A           | the Invention |
| 30 | II-4                | 60 $\mu$ m   | A           | 60 $\mu$ m   | A           | the Invention |
| 30 | II-5                | 60 $\mu$ m   | A           | 60 $\mu$ m   | A           | the Invention |
| 30 | II-6                | 60 $\mu$ m   | A           | 60 $\mu$ m   | A           | the Invention |
| 30 | II-7                | 60 $\mu$ m   | A           | 60 $\mu$ m   | A           | the Invention |
| 30 | II-8                | 60 $\mu$ m   | A           | 60 $\mu$ m   | A           | the Invention |
| 30 | II-9                | 60 $\mu$ m   | A           | 60 $\mu$ m   | A           | the Invention |
| 30 | II-10               | 60 $\mu$ m   | A           | 60 $\mu$ m   | A           | the Invention |
| 30 | II-11               | 60 $\mu$ m   | A           | 60 $\mu$ m   | A           | the Invention |
| 30 | II-12               | 55 $\mu$ m   | B           | 55 $\mu$ m   | B           | the Invention |
| 30 | II-13               | 55 $\mu$ m   | B           | 55 $\mu$ m   | B           | the Invention |
| 30 | II-14               | 55 $\mu$ m   | B           | 55 $\mu$ m   | B           | the Invention |
| 45 | None                | 45 $\mu$ m   | C           | 80 $\mu$ m   | A           | Comp. Example |

TABLE 6

| 50 | <Black Ink>         |              |             |              |             |               |
|----|---------------------|--------------|-------------|--------------|-------------|---------------|
|    | Undercoating Liquid | YUPO 80      |             | N YUPO       |             | Notes         |
|    |                     | Dot diameter | Solid image | Dot diameter | Solid image |               |
| 55 | II-1                | 50 $\mu$ m   | C           | 50 $\mu$ m   | C           | Comp. Example |
| 55 | II-2                | 60 $\mu$ m   | A           | 60 $\mu$ m   | A           | the Invention |
| 55 | II-3                | 60 $\mu$ m   | A           | 60 $\mu$ m   | A           | the Invention |
| 55 | II-4                | 60 $\mu$ m   | A           | 60 $\mu$ m   | A           | the Invention |
| 55 | II-5                | 60 $\mu$ m   | A           | 60 $\mu$ m   | A           | the Invention |
| 55 | II-6                | 60 $\mu$ m   | A           | 60 $\mu$ m   | A           | the Invention |
| 55 | II-7                | 60 $\mu$ m   | A           | 60 $\mu$ m   | A           | the Invention |
| 55 | II-8                | 60 $\mu$ m   | A           | 60 $\mu$ m   | A           | the Invention |
| 55 | II-9                | 60 $\mu$ m   | A           | 60 $\mu$ m   | A           | the Invention |
| 55 | II-10               | 60 $\mu$ m   | A           | 60 $\mu$ m   | A           | the Invention |
| 55 | II-11               | 60 $\mu$ m   | A           | 60 $\mu$ m   | A           | the Invention |
| 55 | II-12               | 55 $\mu$ m   | B           | 55 $\mu$ m   | B           | the Invention |
| 55 | II-13               | 55 $\mu$ m   | B           | 55 $\mu$ m   | B           | the Invention |
| 55 | II-14               | 55 $\mu$ m   | B           | 55 $\mu$ m   | B           | the Invention |

TABLE 6-continued

| <Black Ink>            |                 |                |                 |                |                  |
|------------------------|-----------------|----------------|-----------------|----------------|------------------|
| Undercoating<br>Liquid | Dot<br>diameter | Solid<br>image | Dot<br>diameter | Solid<br>image | Notes            |
| None                   | 45 $\mu$ m      | C              | 80 $\mu$ m      | A              | Comp.<br>Example |

TABLE 7

| <Full Color Image> |                  |        |               |
|--------------------|------------------|--------|---------------|
| Undercoating       | Full color image |        |               |
| Liquid             | YUPO 80          | N YUPO | Notes         |
| II-1               | C                | C      | Comp. Example |
| II-2               | A                | A      | the Invention |
| II-3               | A                | A      | the Invention |
| II-4               | A                | A      | the Invention |
| II-5               | A                | A      | the Invention |
| II-6               | A                | A      | the Invention |
| II-7               | A                | A      | the Invention |
| II-8               | A                | A      | the Invention |
| II-9               | A                | A      | the Invention |
| II-10              | A                | A      | the Invention |
| II-11              | A                | A      | the Invention |
| II-12              | A                | A      | the Invention |
| II-13              | A                | A      | the Invention |
| II-14              | A                | A      | the Invention |
| None               | E                | D      | Comp. Example |

As shown in Tables 3 to 7, in the examples using an oligomer in which adjacent dots are in connection with each other, a clear image with high density without white spots was obtained even when the image is recorded with low resolution such as 300 dpi $\times$ 600 dpi with a small liquid amount such as 24 pL. On the other hand, in the comparative examples using no oligomer, in which spreading of the dots was not sufficient enough for the dots to connect with each other and white spots were caused, and an indistinct or uneven image with low density was formed with such a low resolution.

Further, there was no dependency on the type of substrate in the examples using an undercoating liquid, whereas in the comparative examples without using the undercoating liquid, the manner of adjacent dots connect varied according to the type of the substrate and uniform images could not obtain, and the quality of the images were not sufficiently acceptable.

Accordingly, the invention provides an ink jet recording method and an ink jet recording device in which images can be recorded with high uniformity on various types of recording media, while preventing ink bleeding or unevenness in line width or color due to coalescence of ink droplets. Further, an image can be recorded with high density and reproducibility to details, irrespective of the form of the image.

Therefore, according to the ink jet recording method and an ink jet recording device of the invention, high-quality images with high density clearly reproduced to details can be obtained due to coalescence of adjacent ink droplets over the whole image, even when a low-cost head unit with low resolution is used in a single pass method in which high-speed image formation can be performed.

All publications, patent applications, and technical standards mentioned in this specification are herein incorporated

by reference to the same extent as if each individual publication, patent application, or technical standard was specifically and individually indicated to be incorporated by reference.

What is claimed is:

1. An ink jet recording method comprising:  
applying an undercoating liquid comprising an oligomer and a surfactant onto a recording medium;  
partially curing the undercoating liquid that has been applied onto the recording medium; and  
recording an image by ejecting onto the partially cured undercoating liquid an ink that is curable by irradiation with actinic energy rays, and wherein  
at least one surfactant contained in the undercoating liquid satisfies the following relation (B):

$$\gamma_s(0) - \gamma_s(\text{saturated}) > 0 \text{ (mN/m)},$$

and the surface tension of the undercoating liquid satisfies the following relation (C):

$$\gamma_s < (\gamma_s(0) + \gamma_s(\text{saturated}))^{max}/2$$

wherein,  $\gamma_s$  represents the value of the surface tension of the undercoating liquid;  $\gamma_s(0)$  represents the value of the surface tension of a liquid having a composition of the undercoating liquid from which all surfactants are excluded;  $\gamma_s$  (saturated) represents the value of the surface tension of a liquid, wherein the liquid is obtained by adding one of the surfactants contained in the undercoating liquid to the above "liquid excluding all of the surfactants", the value being measured when the surface tension reaches a point of saturation as the density of the surfactant is increased; and  $\gamma_s$  (saturated)<sup>max</sup> represents the maximum value among the values of  $\gamma_s$  (saturated) respectively measured for all kinds of the surfactants which are contained in the undercoating liquid that satisfies the above relation (B).

2. The ink jet recording method of claim 1, wherein the oligomer is a urethane acrylate oligomer.

3. The ink jet recording method of claim 1, wherein the undercoating liquid is cured by irradiation with actinic energy rays.

4. The ink jet recording method of claim 1, wherein the undercoating liquid further comprises a radical polymerizable composition.

5. The ink jet recording method of claim 1, wherein the image is recorded with a multi-color ink set, and the method further comprises partially curing the ink of at least one color ejected onto the recording medium.

6. The ink jet recording method of claim 1, further comprising promoting the curing of the ink and the undercoating liquid.

7. The ink jet recording method of claim 1, wherein the curing sensitivity of the ink is equal to or higher than the curing sensitivity of the undercoating liquid.

8. The ink jet recording method of claim 1, wherein the internal viscosity at 25 °C. of the partially cured undercoating liquid is at least 1.5 times the viscosity at 25 °C. at the surface of the partially cured undercoating liquid.

9. The ink jet recording method of claim 1, wherein the recording medium is non-permeable or slowly permeable.

10. The ink jet recording method of claim 1, wherein the undercoating liquid is applied by a coater.